



US007306898B2

(12) **United States Patent**  
**Shimada**

(10) **Patent No.:** **US 7,306,898 B2**  
(45) **Date of Patent:** **Dec. 11, 2007**

(54) **PLANOGRAPHIC PRINTING METHOD AND  
PLANOGRAPHIC PRINTING PLATE  
PRECURSOR USED THEREIN**

(75) Inventor: **Kazuto Shimada**, Shizuoka-ken (JP)

(73) Assignee: **Fujifilm Corporation**, Tokyo (JP)

(\*) Notice: Subject to any disclaimer, the term of this patent is extended or adjusted under 35 U.S.C. 154(b) by 0 days.

(21) Appl. No.: **11/050,037**

(22) Filed: **Feb. 4, 2005**

(65) **Prior Publication Data**

US 2005/0191581 A1 Sep. 1, 2005

(30) **Foreign Application Priority Data**

Feb. 20, 2004 (JP) ..... 2004-045114

(51) **Int. Cl.**

**G03F 7/30** (2006.01)

(52) **U.S. Cl.** ..... **430/302**; 430/281.1; 430/286.1;  
430/288.1; 430/309; 430/494; 430/944; 430/945;  
430/138

(58) **Field of Classification Search** ..... 430/138,  
430/270.1, 281.1, 286.1, 287.1, 288.1, 302,  
430/309, 494, 944, 945

See application file for complete search history.

(56) **References Cited**

U.S. PATENT DOCUMENTS

6,143,464 A \* 11/2000 Kawauchi ..... 430/270.1  
6,692,896 B2 \* 2/2004 Shimada et al. ..... 430/281.1  
6,939,658 B2 \* 9/2005 Oohashi et al. ..... 430/163  
2002/0086238 A1 \* 7/2002 Fujimaki et al. ..... 430/281.1  
2002/0102488 A1 \* 8/2002 Yanaka et al. ..... 430/138

2005/0031986 A1 \* 2/2005 Kakino et al. ..... 430/270.1

FOREIGN PATENT DOCUMENTS

|    |               |         |
|----|---------------|---------|
| JP | 2938397 B2    | 6/1999  |
| JP | 2001-277740 A | 10/2001 |
| JP | 2001-277742 A | 10/2001 |
| JP | 2002-287334 A | 10/2002 |

\* cited by examiner

Primary Examiner—Barbara L. Gilliam

(74) Attorney, Agent, or Firm—Birch, Stewart, Kolasch & Birch, LLP

(57) **ABSTRACT**

A planographic printing method including: providing a planographic printing plate precursor including a substrate and an image recording layer which is disposed on the substrate and contains (A) an infrared absorber, (B) a polymerization initiator and (C) a polymerizable compound; imagewise exposing the planographic printing plate precursor with an infrared laser; and supplying oil-based ink and an aqueous component to the exposed planographic printing plate precursor without any development treatment, so as to print an image. A region of the planographic printing plate precursor that has not been exposed with an infrared laser is removed during the printing. The polymerizable compound of (C) is represented by the following formula (1):



Formula (1)

wherein  $\text{Ar}^1$ ,  $\text{R}^1$ ,  $\text{Z}$  and  $n$  are as defined in the claims and the specification.

**18 Claims, No Drawings**

## 1

**PLANOGRAFIC PRINTING METHOD AND  
PLANOGRAFIC PRINTING PLATE  
PRECURSOR USED THEREIN**

**CROSS-REFERENCE TO RELATED  
APPLICATION**

This application claims priority under 35USC 119 from Japanese Patent Application No. 2004-045114, the disclosure of which is incorporated by reference herein.

**BACKGROUND OF THE INVENTION**

**1. Field of the Invention**

The present invention relates to a planographic printing method and a planographic printing plate precursor used therein. Specifically, the invention relates to a planographic printing method of printing a planographic printing plate precursor by direct development in a printing machine without any development treatment step and to a planographic printing plate precursor capable of direct plate-making by scanning an infrared laser on the basis of a digital signal from a computer, etc., which is used preferably in the planographic printing method.

**2. Description of the Related Art**

Generally, a planographic printing plate includes a lipophilic image region receiving ink in a printing step and a hydrophilic non-image region receiving dampening water. Planographic printing is a method wherein the property of repellency between water and oil-based ink is utilized to cause a difference in adhesion of the ink to the surface of the planographic printing plate in which the lipophilic image region serves as an ink receiving part and the hydrophilic non-image region serves as a dampening water receiving part (part not receiving the ink), and the ink is allowed to adhere to only the image region and then transferred to a material to be printed such as paper.

For making such a planographic printing plate, a planographic printing plate precursor (PS plate) having a lipophilic photosensitive resin layer (image recording layer) arranged on a hydrophilic substrate has been widely used. Usually, the planographic printing plate is obtained by a method wherein the planographic printing plate precursor is exposed to light via an original image on a lithographic film or the like, and the image recording layer in the image region is allowed to remain, while the image recording layer in the non-image region is removed by dissolution with an alkali developing solution or an organic solvent, thereby exposing the surface of the hydrophilic substrate to make a printing plate.

In a plate-making process using a conventional planographic printing plate precursor, a step of removing the non-image region by dissolution with a developing solution corresponding to the image recording layer is necessary after exposure to light, and elimination or simplification of such additional wet treatment is mentioned as a task to be achieved. In recent years, disposal of waste liquid discharged in the wet treatment is a matter of high concern for the whole industry in consideration of the global environment, so there is an increasing demand for achieving this task.

In response to this demand, a method called in-machine development wherein an image recording layer from which a non-image region on a planographic printing plate precursor can be removed in an ordinary printing step is used to remove the non-image region in a printing machine after

## 2

exposure to light to provide a planographic printing plate has been proposed as an easy plate-making method.

Specifically, the method of in-machine development includes, for example, a method of using a planographic printing plate precursor having an image recording layer capable of being dissolved or dispersed in dampening water, an ink solvent or an emulsion of ink and dampening water, a method which involves physical removal of an image recording layer by contact with a roller or a blanket cylinder in a printing machine, and a method which involves physical removal of an image recording layer by contact with a roller or a blanket cylinder after weakening either the cohesive force of the image recording layer or the adhesion between the image recording layer and a substrate by permeation with dampening water, an ink solvent, or the like.

Unless otherwise noted, "development treatment step" in the invention refers to a step wherein the region of a planographic printing plate precursor which has not been exposed to light from an infrared laser is removed by contact with a liquid (usually an alkaline developing solution) in an apparatus (usually an automatic developing machine) other than a printing machine, to expose the surface of a hydrophilic substrate, and "in-machine development" refers to a method and process wherein the region of a planographic printing plate precursor which has not been exposed to light from an infrared laser is removed by contact with a liquid (usually printing ink and/or dampening water) in a printing machine.

However, when an image recording layer in a conventional image recording system using ultraviolet rays or visible light is used, the image recording layer is not fixed even after light exposure, thus making it necessary to use a troublesome method wherein the exposed planographic printing plate precursor is stored in a completely shaded state or under thermostatic conditions until it is fitted into a printing machine.

In recent years, digitalization techniques which involve electronic processing, accumulation and output of image information with a computer are spreading, and a wide variety of new image output systems compatible with the digitalization techniques have come to be practically used. As a result, attention has been paid to computer-to-plate (CTP) techniques of producing a planographic printing plate directly by scanning a planographic printing plate precursor with highly directional light such as laser light carrying digitalized image information without using a lithographic film. Accordingly, it is an important technical problem to provide a planographic printing plate precursor adapted to these techniques.

As described above, simplification of a plate-making operation as well as providing a dry, treatment-free plate-making operation has been desired more strongly than in the past because of concern about both the global environment and adaptation to digitalization.

Because high-power lasers such as semiconductor lasers, YAG lasers, and the like have come to be inexpensively available in recent years, a method of using such a high-power laser as an image recording means is regarded as a promising method of producing a planographic printing plate by scanning light which can be easily adapted to digitalization techniques.

The conventional plate-making method involves image-wise exposure to light at low to medium intensity, to record an image by an image-wise change in physical properties due to a photochemical reaction in the image recording layer. On the other hand, the method of using a high-power laser involves emitting a large amount of light energy in a very

3

short time onto a region to be exposed to light, to convert the light energy efficiently into heat energy by which the image recording layer is caused to undergo thermal change such as a chemical change, a phase change, or a change in form or structure, and then utilizing the change in image recording. Accordingly, although the image information is outputted by light energy such as laser light, image recording is conducted not only by light energy but also by heat energy. Usually, the recording system using generation of heat by exposure to high-power density light is called heat mode recording, and conversion of light energy into heat energy is called light/heat conversion.

A great advantage of the plate-making method using heat mode recording is that the image recording layer is not sensitive to light at an ordinary intensity level such as interior illumination, and also that fixation of an image recorded by exposure to high-intensity light is not essential. That is, the planographic printing plate precursor used in heat mode recording is not sensitive to indoor light before light exposure is carried out, and fixation of the resulting image after light exposure is carried out is not essential. Accordingly, the plate-making process wherein an image recording layer to be made insoluble or soluble by exposure to light from a high-power laser is exposed to imagewise light to form a planographic printing plate can be carried out using in-machine development, thereby realizing a printing system wherein the image is not influenced even by exposure to indoor ambient light. Accordingly, it is expected that a planographic printing plate precursor used preferably in in-machine development can be obtained by utilizing heat mode recording.

The development of lasers in recent years has been remarkable, and in particular, high-power, small-size solid lasers and semiconductor lasers emitting infrared rays of wavelengths of 760 to 1200 nm can be easily obtained. These infrared lasers are very useful as recording light sources for direct plate-making by digital data from computers, etc.

However, many photosensitive recording materials that are practically useful as the image recording layer have photosensitive wavelengths in the visible light range of 760 nm or less, and therefore cannot be used in recording an image with an infrared laser. Accordingly, there is a need for materials capable of image recording with an infrared laser.

As such an image recording material, a planographic printing plate precursor having a hydrophilic substrate on which an image recording layer comprising hydrophobic thermoplastic polymer particles dispersed in a hydrophilic binder is arranged has been proposed in Japanese Patent No. 2938397. This planographic printing plate precursor can be exposed to light from an infrared laser to thermally fuse the hydrophobic thermoplastic polymer particles to form an image, fitted onto a cylinder in a printing machine, and subjected to in-machine development with dampening water and/or ink, and exhibits good in-machine development properties. However, in the method of forming an image in this manner by mere thermal fusion of fine particles, there is a problem in that the image intensity, and particularly the adhesiveness of the substrate to the ink receiving layer, is very low, and printing durability is insufficient.

As other examples of such planographic printing plate precursors that can be subjected to in-machine development, a planographic printing plate precursor containing micro-capsules incorporating a polymerizable compound on a hydrophilic substrate (see, for example, Japanese Patent Application Laid-Open (JP-A) Nos. 2001-277740 and 2001-277742) and a planographic printing plate precursor pro-

4

vided with a photosensitive layer containing an infrared absorber, a radical polymerization initiator and a polymerizable compound on a substrate (see, for example, JP-A No. 2002-287334) have been proposed.

5 An image region produced by the method of forming an image in this manner by polymerization reaction has a higher density of chemical bonds in the image region than in an image region formed by thermal fusion of fine polymer particles and is thus inherently relatively excellent in image density. However, from a practical standpoint, the method of using a polymerization reaction is still insufficient in in-machine development properties, printing durability and polymerization efficiency (sensitivity) and is not practically usable.

## SUMMARY OF THE INVENTION

The present invention has been made in view of the above-described circumstances and provides a planographic printing method capable of giving a large number of excellent prints with a practical amount of energy by using a planographic printing plate precursor capable of recording an image by a laser emitting infrared rays, thereby recording an image by exposure to infrared laser rays directly from digital data from a computer, etc., and subsequent in-machine development in a printing step without any development treatment step. The invention further provides a planographic printing plate precursor used preferably in the planographic printing method of the invention.

In order to achieve the foregoing, the inventors paid attention to constituent components in a negative-type image recording material used in an image recording layer in a planographic printing plate precursor, and they selected a specific compound as a polymerizable compound, and the invention was thereby completed.

A first aspect of the present invention is to provide a planographic printing method comprising: providing a planographic printing plate precursor comprising a substrate 40 and an image recording layer which is disposed on the substrate and comprises (A) an infrared absorber, (B) a polymerization initiator and (C) a polymerizable compound, the image recording layer being capable of recording with irradiation of infrared rays; imagewise exposing the planographic printing plate precursor with an infrared laser; and 45 supplying oil-based ink and an aqueous component to the exposed planographic printing plate precursor without any development treatment, so as to print an image.

50 A region of the planographic printing plate precursor that has not been exposed with an infrared laser is removed during the printing, and the polymerizable compound of (C) is represented by the following formula (1):



Formula (1)

wherein  $\text{Ar}^1$  represents an arylene group or a divalent heterocyclic group;  $\text{R}^1$  represents a hydrogen atom or an alkyl group having 1 to 6 carbon atoms;  $\text{Z}$  represents an  $n$ -valent organic linking group; and  $n$  denotes an integer of 1 to 20.

## 5

In a preferable embodiment of the planographic printing method of the invention, the polymerization initiator of (B) contained in the image recording layer is an onium salt.

Preferably, the image recording layer further comprises (D) a binder polymer.

In view of image formability and removability of a non-image, the image recording layer preferably comprises (F) microcapsules. The microcapsules preferably incorporate at least one of the components contained in the image recording layer.

An acrylic monomer is preferably used as a polymerizable compound in a system of forming an image through curing by radical polymerization such as in the image recording layer of the invention. This acrylic monomer is highly reactive and effective in improving sensitivity, but contains a relatively high hydrophilic ester group and is often highly hydrophilic because a part of functional group upon rendered multifunctional remains as hydroxyl group. Accordingly, an image region may be damaged by dampening water, etc. during printing to deteriorate printing durability. There easily occurs the influence of dampening water on the printing durability of an image region of particularly small area such as halftone dots and thin lines, but in the invention, a highly hydrophobic styrene-based monomer represented by formula (1) is used as the polymerizable compound, and thus dampening water can be prevented from exerting an influence on the image region after curing, whereby printing durability is improved, and this effect is significant in particular in an image region of small area such as halftone dots.

On the other hand, the unexposed regions, that is, the non-image regions, have a slightly higher hydrophilicity compared to that of other polymerizable compounds. However, the unexposed regions are easily removed with ink or the like during printing, and thus it is possible to secure development properties at the same level to conventionally used hydrophilic acrylic monomers.

According to the planographic printing method of the invention, an image excellent in reproducibility of an image region of small area such as halftone dots and fine lines can be obtained, while high on-machine development properties can be secured.

A second aspect of the present invention is to provide a planographic printing plate precursor comprising a substrate and an image recording layer which is disposed on the substrate and comprises (A) an infrared absorber, (B) a polymerization initiator and (C) a polymerizable compound, the image recording layer being removable with printing ink and/or dampening water. The polymerizable compound of (C) is represented by the following formula (1):

Formula (1)



wherein  $Ar^1$  represents an arylene group or a divalent heterocyclic group;  $R^1$  represents a hydrogen atom or an alkyl group having 1 to 6 carbon atoms;  $Z$  represents an  $n$ -valent organic linking group; and  $n$  denotes an integer of 1 to 20.

## 6

The polymerization initiator of (B) contained in the image recording layer of the planographic printing plate precursor is preferably an onium salt.

Other components that can be added optionally to the image recording layer include (D) a binder polymer and (F) microcapsules. The microcapsules (F) may incorporate at least one of the components contained in the image recording layer.

10 According to the planographic printing method of the invention, a large number of excellent prints, particularly prints excellent in halftone dot reproducibility, can be obtained with a practical amount of energy by using a planographic printing plate precursor capable of recording 15 an image by a laser emitting infrared rays, thereby recording an image by exposure to infrared laser rays directly from digital data from a computer, etc., followed by in-machine development in a printing step without any development 20 treatment step.

25 The planographic printing plate precursor of the invention is excellent in printing durability of an image region and removability of a non-image region and can be preferably used in a planographic printing method where in-machine development is carried out, and the resulting print is excellent in reproducibility of halftone dots.

DETAILED DESCRIPTION OF THE  
INVENTION

30 Hereinafter, the present invention is described in more detail.

35 The planographic printing method of the invention comprises: providing a planographic printing plate precursor comprising a substrate and an image recording layer which is disposed on the substrate and comprises (A) an infrared absorber, (B) a polymerization initiator and (C) a polymerizable compound. The polymerizable compound of (C) is represented by the above-described formula (1). The image recording layer is capable of recording with irradiation of 40 infrared rays. Hereinafter, the structure of the planographic printing plate precursor used preferably in the planographic printing method of the invention is described in detail.

[Planographic Printing Plate Precursor]

<Image Recording Layer>

50 The image recording layer in the planographic printing plate precursor of the invention comprises (A) an infrared absorber, (B) a polymerization initiator and (C) a polymerizable compound represented by the above-described formula (1), and preferably further comprises a binder polymer (D).

55 In the planographic printing plate precursor of the invention, a light-exposed portion of the image recording layer is cured by irradiation with infrared rays to form a hydrophobic (lipophilic) region, and when printing is initiated, a region not exposed to light is rapidly removed from a substrate by dampening water, ink, or an emulsion of ink and dampening water. That is, the image recording layer is an image recording layer removable with printing ink and/or dampening water. Hereinafter, each component of the image recording layer is described in detail.

<(C) Polymerizable Compound Represented by Formula (1)>

The polymerizable compound which is a characteristic component of the invention is described. The polymerizable compound used in the invention is a compound represented by the following formula (1) (hereinafter, sometimes referred to as compound (C)):



Formula (1)

In formula (1), Ar¹ represents an arylene group or a divalent heterocyclic group. R¹ represents a hydrogen atom or an alkyl group having 1 to 6 carbon atoms. Zn is an n-valent organic linking group. n is an integer of 1 to 20. When n is 1, Z is not a linking group but a substituent group of Ar¹.

In formula (1), Ar¹ represents an arylene group or a divalent heterocyclic group. Examples of the ring constituting the arylene group include a benzene ring, a condensed ring formed by 2 to 3 benzene rings, and a condensed ring formed by a benzene ring and a 5-membered unsaturated ring. Specific examples of the arylene group include a carbon cyclic divalent group such as a benzene ring, naphthalene ring, anthracene ring, phenanthrene ring, indene ring, acenaphthylene ring and fluorene ring. Examples of the divalent heterocyclic group include a group having 3 to 20 carbon atoms and a group containing 1 to 5 heteroatoms. Specific examples include heterocyclic divalent groups such as a quinoline ring, benzofuran ring, thioxanthone ring, carbazole ring, indole ring, benzofuran ring, imidazole ring, etc. which have a carbon ring such as a pyridine ring, furan ring, and benzene ring condensed with a heterocyclic ring.

Ar¹ may have a substituent group, and examples of such a substituent group include monovalent nonmetallic atomic groups excluding hydrogen. Specific examples of the substituent group include halogen atoms (F, Cl, Br, I), a hydroxy group, cyano group, nitro group, formyl group, C<sub>1</sub> to C<sub>12</sub> linear, branched or cyclic alkyl group, alkenyl group, alkynyl group, carbonyl group, alkoxy group, aryloxy group, carbonyl group, alkoxythio group, arylthio group, amino group, phenyl group, naphthyl group, sulfoxy group, sulfonyl group, carbamoyl group, sulfamoyl group and substituent groups obtained by combining these substituent groups. Examples of these substituent groups include a n-butyl group, s-butyl group, t-butyl group, dodecyl group, cyclohexyl group, trifluoromethyl group, chloromethyl group, bromophenyl group, mesityl group, vinyl group, cinnamyl group, cyclopentene group, 1-propenyl group, ethynyl group, acetyl group, carboxyphenyl group, acetoxy group, ethoxycarbonyl group, methoxy group, n-butoxy group, methylthiomethyl group, phenoxy group, diethylamino group, diphenylamino group, methylphenylamino group, methoxymethyl group, benzyl group, acetylaminogroup, acetylaminooethyl group, methoxysulfonyl group, ethylsulfoxy group, phenylsulfonyl group, carbamoylmethyl group, etc. Among these substituent groups, more preferable groups include an alkyl group, alkenyl group, alkynyl group, halogen atom, hydroxy group and alkoxy group.

When Ar¹ represents a substituted arylene group or a divalent heterocyclic group, examples of Ar¹ include divalent groups such as biphenyl, tolyl, xylyl, mesityl, cumenyl,

chlorophenyl, bromophenyl, fluorophenyl, chloromethylphenyl, trifluoromethylphenyl, hydroxyphenyl, methoxyphenyl, methoxyethoxyphenyl, allyloxyphenyl, phenoxysubstituted phenyl, methylthiophenyl, tolylthiophenyl, ethylaminophenyl, diethylaminophenyl, morpholinophenyl, acetoxyphenyl, benzoyloxyphenyl, N-cyclohexylcarbamoyloxyphenyl, N-phenylcarbamoyloxyphenyl, acetylaminophenyl, N-methylbenzoylaminophenyl, carboxyphenyl, methoxycarbonylphenyl, allyloxy carbonylphenyl, chlorophenoxy carbonylphenyl, carbamoylphenyl, N-methylcarbamoylphenyl, N,N-dipropylcarbamoylphenyl, N-(methoxyphenyl) carbamoylphenyl, N-methyl-N-(sulfonylphenyl) carbamoylphenyl, sulfophenyl, sulfonatophenyl, sulfamoylphenyl, N-ethylsulfamoylphenyl, N,N-dipropylsulfamoylphenyl, N-tolylsulfamoylphenyl, N-methyl-N-(phosphonophenyl) sulfamoylphenyl, phosphonophenyl, phosphonatophenyl, diethylphosphonophenyl, diphenylphosphonophenyl, methylphosphonophenyl, methylphosphonatophenyl, tolylphosphonophenyl, tolylphosphonatophenyl, allylphenyl group, 1-propenylmethylphenyl group, 2-but enylphenyl group, 2-methylallylphenyl, 2-methylpropenylphenyl, 2-propynylphenyl, 2-butynylphenyl, 3-butynylphenyl, etc.

Ar¹ is preferably an arylene group which does not have a substituent group, and is particularly preferably a phenylene group.

In formula (1), R¹ represents a hydrogen atom or an alkyl group having 1 to 6 carbon atoms. The alkyl group may be linear or branched. In particular, a methyl group and ethyl group are preferable.

It is preferable that the compound (C) is multifunctional, because binding of the polymerizable compounds or sites crosslinking with a binder are increased, thereby significantly improving the efficiency of crosslinking reaction and further improving printing durability as the effect of the invention.

In formula (1), Z is an n-valent organic linking group. Insofar as the organic linking group is an n-valent organic group, it is not particularly limited and can be constituted so as to contain the following functional group. Examples of such a functional group include any group selected from a group of divalent groups shown below, an alkyl group, alkenyl group, alkynyl group, benzyl group, aryl group, and a divalent group including a combination of 2 or more groups selected from a group of divalent groups shown below.



In the above formulae, Ar represents an arylene group, and R and R' each independently represent an alkyl group, an alkenyl group or an aryl group.

Z is more preferably an n-valent organic linking group containing at least one of the following groups:



n is an integer of 1 to 20. n is preferably 2 or more, and more preferably 3 or more. Z is defined as an n-valent organic linking group. However, when n is 1, Z represents a substituent group of Ar<sup>1</sup>.

The positions of Z- and CH<sub>2</sub>=CR<sup>1</sup>— with which Ar<sup>1</sup> is substituted are not particularly limited, but in view of easiness of synthesis, CH<sub>2</sub>=CR<sup>1</sup>— is preferably at a para-position with respect to Z-.

For the sake of convenience, examples of the compound to be preferably used as compound (C) are classified into groups I to VI according to their structural characteristics, and each group is further classified into group (a) (not having a heteroatom) and group (b) (having a heteroatom), as shown below. However, these examples should not be construed to limit the compound (C) used in the invention.

### Group I

| Group I-(a) |                    |                                                   | Group I-(b) |                |                                                      |
|-------------|--------------------|---------------------------------------------------|-------------|----------------|------------------------------------------------------|
| I-(a)-(i)-  | R <sup>2</sup>     | R <sup>3</sup>                                    | I-(b)-(i)-  | R <sup>8</sup> | R <sup>9</sup>                                       |
| 1           | —H                 | —H                                                | 1           | —H             | —OH                                                  |
| 2           | —H                 | —Me                                               | 2           | —H             | —O— <sup>n</sup> Bu                                  |
| 3           | —H                 | — <sup>t</sup> Bu                                 | 3           | —H             | —O—CH(CH <sub>3</sub> ) <sub>2</sub>                 |
| 4           | —H                 | —(CH <sub>2</sub> ) <sub>11</sub> CH <sub>3</sub> | 45          | —H             | —OC—C <sub>2</sub> H <sub>5</sub><br>CH <sub>3</sub> |
| 5           | —H                 | —CH=CH <sub>2</sub>                               | 46          | 5              | —H                                                   |
| 6           | —Me                | —H                                                | 6           | —H             | —O— <sup>t</sup> Bu                                  |
| 7           | —Me                |                                                   | 50          | 7              | —H                                                   |
| 8           | —Me                | —Me                                               | 8           | —H             | —COCH <sub>3</sub>                                   |
| 9           | —Me                | — <sup>t</sup> Bu                                 | 9           | —H             | —SO <sub>2</sub> OCH <sub>3</sub>                    |
| 10          | —Et                | —H                                                | 10          | —H             | —CO <sub>2</sub> CH <sub>3</sub>                     |
| 11          | — <sup>n</sup> Hex | —H                                                | 11          | —H             | —OSO <sub>2</sub> — <sup>n</sup> Bu                  |
| (ii)        |                    |                                                   | 12          | —H             | —OCO-Ph                                              |
|             |                    |                                                   | 13          | —H             | —COSCH <sub>3</sub>                                  |
|             |                    |                                                   | 14          | —H             | —NH <sub>2</sub>                                     |
|             |                    |                                                   | 15          | —H             | —NHCONH— <sup>n</sup> Bu                             |
|             |                    |                                                   | 16          | —H             | —OCONH-c-Hex                                         |
|             |                    |                                                   | 17          | —H             | —CH <sub>2</sub> O-n-Hex                             |
|             |                    |                                                   | 18          | —H             | —CH <sub>2</sub> S—Et                                |
|             |                    |                                                   | 19          | —H             | —CH <sub>2</sub> OCO-Ph                              |
|             |                    |                                                   | 20          | —H             | —Cl                                                  |
|             |                    |                                                   | 21          | —H             | —F                                                   |
|             |                    |                                                   | 22          | —H             | —OH                                                  |
|             |                    |                                                   | 65          | 23             | —Me                                                  |
|             |                    |                                                   | 24          | —Me            | —CH <sub>2</sub> O— <sup>n</sup> Bu                  |
|             |                    |                                                   | 25          | —Me            | —COCH <sub>3</sub>                                   |

### 10

-continued

|   |             |                                    |
|---|-------------|------------------------------------|
| 5 | Group I-(a) |                                    |
| 5 | —Me         | —CH(CH <sub>3</sub> ) <sub>2</sub> |
| 6 | —Me         | —CH=CH <sub>2</sub>                |

(iii)



|    |              |                     |                |
|----|--------------|---------------------|----------------|
| 15 | I-(a)-(iii)- | R <sup>6</sup>      | R <sup>7</sup> |
| 1  | —H           | —Me                 |                |
| 2  | —H           | —Et                 |                |
| 3  | —H           | —CH=CH <sub>2</sub> |                |
| 4  | —Me          | —Me                 |                |

### Group I-(b)

(i)

|    |            |                |                |
|----|------------|----------------|----------------|
| 30 | I-(b)-(i)- | R <sup>8</sup> | R <sup>9</sup> |
| 35 | 35         |                |                |
| 40 | I-(b)-(i)- | R <sup>8</sup> | R <sup>9</sup> |
| 45 | 45         |                |                |
| 50 | 50         |                |                |
| 55 | 55         |                |                |
| 60 | 60         |                |                |
| 65 | 65         |                |                |
| 70 | 70         |                |                |
| 75 | 75         |                |                |
| 80 | 80         |                |                |
| 85 | 85         |                |                |
| 90 | 90         |                |                |
| 95 | 95         |                |                |

**11**  
-continued

| Group I-(b) |     |          |
|-------------|-----|----------|
| 23          | —Me | —NHCO-Ph |
| 24          | —Me | —Cl      |
| 25          | —Me | —Br      |



(ii)

| I-(b)-(ii)- | R <sup>10</sup> | R <sup>11</sup>                                      |
|-------------|-----------------|------------------------------------------------------|
| 1           | —H              | —OH                                                  |
| 2           | —H              | —O— <sup>n</sup> Bu                                  |
| 3           | —H              | —COCH <sub>3</sub>                                   |
| 4           | —H              | —NHCO-Ph                                             |
| 5           | —H              | —CH <sub>2</sub> O—Et                                |
| 6           | —H              | —Cl                                                  |
| 7           | —Me             | —OH                                                  |
| 8           | —Me             | —O—CH <sub>2</sub> CH(CH <sub>3</sub> ) <sub>2</sub> |
| 9           | —Me             | —F                                                   |
| 10          | —Me             | —Br                                                  |



(iii)

| I-(b)-(iii)- | R <sup>12</sup> | R <sup>13</sup>        |
|--------------|-----------------|------------------------|
| 1            | —H              | —OH                    |
| 2            | —H              | —NH <sub>2</sub>       |
| 3            | —H              | —OCOCH <sub>3</sub>    |
| 4            | —H              | —Br                    |
| 5            | —Me             | —OH                    |
| 6            | —Me             | —NHCO— <sup>n</sup> Bu |
| 7            | —Me             | —F                     |



(iv)

| I-(b)-(iv)- | R <sup>14</sup> | R <sup>15</sup> | R <sup>16</sup>    |
|-------------|-----------------|-----------------|--------------------|
| 1           | —H              | —OH             | —COCH <sub>3</sub> |
| 2           | —H              | —Cl             | —OH                |
| 3           | —H              | —Br             | —NH <sub>2</sub>   |

**12**  
-continued

| Group I-(b) |   |                                               |
|-------------|---|-----------------------------------------------|
| 5           | 4 | —H      —COCH <sub>3</sub> —COCH <sub>3</sub> |
|             | 5 | —Me      —OH      —COCH <sub>3</sub>          |

(v)

| I-(b)-(v)- | R <sup>17</sup> | R <sup>18</sup>    | R <sup>19</sup>      |
|------------|-----------------|--------------------|----------------------|
| 1          | —H              | —OH                | —F                   |
| 2          | —H              | —COCH <sub>3</sub> | —CH <sub>3</sub>     |
| 3          | —H              | —Cl                | —NHCOCH <sub>3</sub> |

(vi)

| I-(b)-(vi)- | R <sup>20</sup> | R <sup>21</sup>     | R <sup>22</sup>     |
|-------------|-----------------|---------------------|---------------------|
| 1           | —H              | —CH <sub>2</sub> OH | —CH <sub>2</sub> OH |
| 2           | —H              | —F                  | —F                  |
| 3           | —H              | —F                  | —CH <sub>3</sub>    |

(vii)

| I-(b)-(vii)- | R <sup>23</sup> | R <sup>24</sup>      | R <sup>25</sup>  |
|--------------|-----------------|----------------------|------------------|
| 1            | —H              | —OH                  | —OH              |
| 2            | —H              | —NHCOCH <sub>3</sub> | —OH              |
| 3            | —Me             | —O— <sup>n</sup> Bu  | —NH <sub>2</sub> |

(viii)

| I-(b)-(viii)- | R <sup>26</sup> | R <sup>27</sup>     | R <sup>28</sup>  |
|---------------|-----------------|---------------------|------------------|
| 1             | —H              | —OH                 | —OH              |
| 2             | —Me             | —O— <sup>n</sup> Bu | —NH <sub>2</sub> |

**13**

-continued

Group I-(b)

(ix)

5



I-(b)-(ix)-

1

2

R29

—H

—Me

10

(x)

I-(b)-(x)-1



20

(xi)

I-(b)-(xi)-1



30

Group II

35

Group II-(a)

(i)



II-(a)-(i)-

X1

45

1 —CH2—

2 —(CH2)4—

3



4



5



6



50

55

**14**

-continued

Group II-(a)

7



8



9



10



(ii)



II-(a)-(ii)-

X2

1 —CH2—

2 —(CH2)4—

3



4



5



6



(iii)

II-(a)-(iii)-

X3

1 —CH2—

2



**15**

| -continued                                                                          |      |
|-------------------------------------------------------------------------------------|------|
| Group II-(a)                                                                        |      |
|                                                                                     | 5    |
|    | (iv) |
| II-(a)-(iv)- X <sup>4</sup>                                                         | 10   |
| 1 $-(CH_2)_4-$                                                                      | 15   |
| 2  | 20   |
|                                                                                     | 25   |
| Group II-(b)                                                                        |      |
|                                                                                     | (i)  |
|   | 30   |
| II-(b)-(i)- X <sup>5</sup>                                                          |      |
| 1 $-CH_2OCO(CH_2)_7CO_2CH_2-$                                                       | 35   |
| 2 $-CH_2O(CH_2)_{12}O-$                                                             |      |
| 3 $-CH_2S(CH_2)_4S-$                                                                |      |
| 4 $-\overline{CH_2OCH_2CH(CH_2)_2OCH_2}-$<br> <br>CH <sub>3</sub>                   | 40   |
| 5 $-CH_2O(CF_2)_2OCH_2-$                                                            |      |
| 6 $-CH_2OSO_2(CH_2)_4SO_2OCH_2-$                                                    |      |
| 7 $-\overline{CH_2OC(CH_2)_4COCH_2}-$<br>  <br>S      S                             | 45   |
| 8 $-CH_2NH(CH_2)_2NHCH_2-$                                                          |      |
| 9 $-CH_2NH(CH_2)_2O-$                                                               |      |
| 10 $-\overline{CH_2N(CH_2)_2N}-$<br>        <br>CH <sub>3</sub> CH <sub>3</sub>     | 50   |
| 11 $-CH_2SO_2(CH_2)_2SO_2CH_2-$                                                     |      |
| 12 $-\overline{CH_2O}-$<br> <br>cyclohexane<br> <br>OCH <sub>2</sub> -              |      |
| 13 $-\overline{CH_2O}-$<br> <br>cyclohexane<br> <br>OCH <sub>2</sub> -              | 60   |
| 14 $-\overline{CH_2O}-$<br> <br>cyclohexane<br> <br> <br> <br>OCH <sub>2</sub> -    |      |

**16**

| -continued                                                                              |      |
|-----------------------------------------------------------------------------------------|------|
| Group II-(b)                                                                            |      |
|                                                                                         | 15   |
|       |      |
| 16    | 10   |
| 17    | 15   |
| 18    | 20   |
| 19    | 25   |
|                                                                                         | (i)  |
|      | 30   |
| 20   | 35   |
| 21  | 40   |
| 22  | 45   |
| 23  | 50   |
| 24  | 55   |
| 25  | 60   |
|                                                                                         | (ii) |
|     | 65   |
| II-(b)-(ii)- X <sup>6</sup>                                                             |      |
| 1 $-\overline{CO(CH_2)_2CO}-$                                                           |      |
| 2 $-\overline{CO(CH_2)_{12}CO}-$                                                        |      |

| -continued   |  |
|--------------|--|
| Group II-(b) |  |
| 3            |  |
| 4            |  |
| 5            |  |
| 6            |  |
| 7            |  |
| 8            |  |
| 9            |  |
| 10           |  |
| 11           |  |
| 12           |  |
| 13           |  |
| 14           |  |
| 15           |  |
| 16           |  |
| 17           |  |
| 18           |  |
| 19           |  |
| 20           |  |
| 21           |  |
| 22           |  |

| -continued   |  |
|--------------|--|
| Group II-(b) |  |
| 5            |  |
| 10           |  |
| 15           |  |
| 20           |  |
| 21           |  |
| 25           |  |
| 30           |  |
| 35           |  |
| 40           |  |
| 45           |  |
| 50           |  |
| 55           |  |
| 60           |  |
| 65           |  |

II-(b)-(iii)-

X<sup>7</sup>

(iii)

**19****20**

-continued

-continued

Group II-(b)

Group II-(b)

16



5



10



II-(b)-(iv)- X8

15



20



II-(b)-(vi)- X10

25



35

(v)



40



II-(b)-(v)- X9

45



50



II-(b)-(vii)- X11

55



60



65



**21****22**

-continued

-continued

Group II-(b)

Group II-(b)

(viii) 5

10



10



II-(b)-(viii)-

Ar3

15

11



20



2



25



3



30

13



35



5



40

14



6



45

15



7



50

16



8



55

16

9



60



II-(b)-(ix)-

Ar4

(ix)

65

II-(b)-(ix)-

Ar4

-continued

## Group II-(b)



## Group III

5

-continued

## Group III-(a)



15



20



25



30



35

40



45



6



7



8

## Group III-(a)

50



55



60

65

-continued



-continued

-continued

Group III-(b)

Group III-(b)



5

10

15

III-(b)-  $X^{13}$ 

20

25

30 Group IV

35

40

45

50

55

60

65



-continued

## Group IV-(a)



- 6 
- 7 
- 8 
- 9 

5

10

15

20

25

30

35

40

45

50

55

60

65

-continued

## Group IV-(b)



- 7  $-(CO_2CH_2)_4C-$



- 9  $-(CO_2CH_2)_3C-CH_2OCH_2-$



Group IV-(a)

5

IV-(a)

Group VI-(b)

VI-(b)-

1



-continued

Group VI-(b)

VI-(b)-



Among the compounds illustrated in the above, the illustrated compounds having two or more styrene groups in groups II to VI are preferable, and the illustrated compounds having three or more styrene groups in groups III to VI are more preferable. Among the illustrated compounds in groups I to IV, the illustrated compounds in group (b) wherein the linking group Z has a heteroatom are preferable in respect of solubility and development properties.

In view of the film strength of an image region, compound (C) is preferably contained in the image recording layer in an amount of 5 to 70% by mass, and more preferably 10 to 65% by mass, based on the mass of the solid content of the image recording layer of the invention.

Compound (C) in the image recording layer of the invention may be used alone or as a mixture of two or more thereof. Compound (C) only may be used as the polymerizable compound, or may be used in combination with other polymerizable compounds described later in such a range that the effect of the invention is not hindered. When compound (C) is used in combination with other polymerizable compounds, the amount of the other polymerizable compounds is preferably 50 wt % or less relative to the total polymerizable compounds.

## Usable Polymerizable Compound

The other polymerizable compound which can be used in combination with compound (C) in the invention is preferably an addition-polymerizable compound having at least one ethylenically unsaturated double bond, and is selected preferably from compounds each having at least one (preferably two or more) ethylenically unsaturated bond. A group of such compounds is known widely in this industrial field, and in the invention, these compounds can be used without

any particular limitation. These compounds occur in chemical forms such as monomers, prepolymers, that is, dimers, trimers and oligomers, as well as mixtures and copolymers thereof.

Examples of such monomers and copolymers include unsaturated carboxylic acids (e.g., acrylic acid, methacrylic acid, itaconic acid, crotonic acid, isocrotonic acid, maleic acid, etc.) and esters and amides thereof, and preferably used among these compounds are esters between unsaturated carboxylic acids and aliphatic polyvalent alcohols and amides between unsaturated carboxylic acids and aliphatic polyvalent amines. Also preferably used among these compounds are unsaturated carboxylates having nucleophilic substituent groups such as hydroxyl group, amino group, mercapto group, etc., addition-reaction products of amides with monofunctional or multifunctional isocyanates or epoxy compounds, and dehydration condensation reaction products of amides with monofunctional or multifunctional carboxylic acids.

Also preferably used among these compounds are unsaturated carboxylates having electrophilic substituent groups such as isocyanate group, epoxy group, etc., addition-reaction products of amides with monofunctional or multifunctional alcohols, amines or thiols, unsaturated carboxylates having eliminating substituent groups such as halogen group, tosylate group, etc., and substitution-reaction products of amides with monofunctional or multifunctional alcohols, amines or thiols. Use can also be made of a group of those compounds wherein the above-described carboxylic acids have been replaced by unsaturated phosphonic acids, styrene, vinyl ethers, etc.

As the ester monomers of aliphatic polyvalent alcohols and unsaturated carboxylic acids, examples of the acrylates include ethylene glycol diacrylate, triethylene glycol diacrylate, 1,3-butane diol diacrylate, tetramethylene glycol diacrylate, propylene glycol diacrylate, neopentyl glycol diacrylate, trimethylol propane triacrylate, trimethylol propane tri(acryloyloxypropyl)ether, trimethylol ethane triacrylate, hexane diol diacrylate, 1,4-cyclohexane diol diacrylate, tetraethylene glycol diacrylate, pentaerythritol diacrylate, pentaerythritol triacrylate, pentaerythritol tetracrylate, dipentaerythritol diacrylate, dipentaerythritol hexacrylate, sorbitol triacrylate, sorbitol tetracrylate, sorbitol pentacrylate, sorbitol hexacrylate, tri(acryloyloxyethyl) isocyanurate, polyester acrylate oligomers, etc.

Examples of the methacrylates include tetramethylene glycol dimethacrylate, triethylene glycol dimethacrylate, neopentyl glycol dimethacrylate, trimethylol propane trimethacrylate, trimethylol ethane trimethacrylate, ethylene glycol dimethacrylate, 1,3-butane diol dimethacrylate, hexane diol dimethacrylate, pentaerythritol dimethacrylate, pentaerythritol trimethacrylate, pentaerythritol tetramethacrylate, dipentaerythritol dimethacrylate, dipentaerythritol hexamethacrylate, sorbitol trimethacrylate, sorbitol tetramethacrylate, bis[p-(3-methacryloxy-2-hydroxypropoxy)phenyl]dimethyl methane, bis[p-(methacryloxyethoxy)phenyl]dimethyl methane, etc.

Examples of the itaconates include ethylene glycol diitaconate, propylene glycol diitaconate, 1,3-butane diol diitaconate, 1,4-butane diol diitaconate, tetramethylene glycol diitaconate, pentaerythritol diitaconate, sorbitol tetraitaconate, etc.

Examples of the crotonates include ethylene glycol dicrotonate, tetramethylene glycol dicrotonate, pentaerythritol dicrotonate, sorbitol tetradicrotonate, etc.

Examples of the isocrotonates include ethylene glycol diisocrotonate, pentaerythritol diisocrotonate, sorbitol tetraisocrotonate, etc.

Examples of the maleates include ethylene glycol dimaleate, triethylene glycol dimaleate, pentaerythritol dimaleate, sorbitol tetramaleate, etc.

Examples of other preferably used esters include aliphatic alcohol-based esters described in JP-B 46-27926, JP-B 51-47334 and JP-A No. 57-196231, those having an aromatic skeleton described in JP-A Nos. 59-5240, 59-5241 and 2-226149, and those having an amino group described in JP-A No. 1-165613. The ester monomers can also be used as a mixture.

As the monomers, examples of the amides of aliphatic polyvalent amines and unsaturated carboxylic acids include e.g. methylene bis-acrylamide, methylene bis-methacrylamide, 1,6-hexamethylene bis-acrylamide, 1,6-hexamethylene bis-methacrylamide, diethylene triamine trisacrylamide, xylylene bisacrylamide, xylylene bismethacrylamide, etc.

Preferable examples of other amide type monomers include those having a cyclohexylene structure described in JP-B 54-21726.

Urethane type addition-polymerizable compounds produced by addition reaction between isocyanates and hydroxyl groups are also preferable, and examples thereof include vinyl urethane compounds containing two or more polymerizable vinyl groups in one molecule, which are prepared by adding vinyl monomers containing a hydroxyl group shown in formula (2) below to polyisocyanates having two or more isocyanate groups in one molecule as described in JP-B 48-41708.

Formula (2)



In formula (2), R and R' each independently represent H or  $\text{CH}_3$ .

10 Urethane acrylates described in JP-A No. 51-37193, JP-B No. 2-32293 and JP-B No. 2-16765 and urethane compounds having an ethylene oxide-type skeleton described in JP-B No. 58-49860, JP-B No. 56-17654, JP-B No. 62-39417 and JP-B No. 62-39418 are also preferable.

15 Addition-polymerizable compounds having an amino structure or sulfide structure in the molecule as described in JP-A Nos. 63-277653, 63-260909 and 1-105238 can be used to prepare photopolymerizable compositions extremely excellent in photosensitizing speed.

20 Other examples include multifunctional acrylates and methacrylates such as polyacrylates and epoxy acrylates obtained by reacting epoxy resin with (meth)acrylic acid as described in JP-A No. 48-64183, JP-B No. 49-43191 and JP-B No. 52-30490. Specific unsaturated compounds described in JP-B No. 46-43946, JP-B No. 1-40337 and JP-B No. 1-40336 and vinyl phosphonic acid-type compounds described in JP-A No. 2-25493 can also be mentioned. In some cases, a structure containing a perfluoroalkyl group described in JP-A 61-22048 is preferably used. Photocuring monomers and oligomers described in the Journal of The Adhesion Society of Japan, vol. 20, No. 7, pp. 300-308 (1984) can also be used.

25 How these addition-polymerizable compounds such as compound (C) in the invention are used, that is, what structure is used, whether they are used singly or in combination, and in which amount they are used, can be arbitrarily determined depending on final performance design. For example, they may be selected according to the following aspects. In respect of photosensitizing speed, their structure preferably has many unsaturated groups in one molecule, and in many cases, they are preferably bifunctional or more. To increase the strength of an image region, i.e. a cured layer, they are preferably trifunctional or more. It is also effective to use a method of regulating both 30 photosensitivity and strength by combined use of compounds (e.g. acrylates, methacrylates, styrene type compounds, and vinyl ether type compounds) having different functionalities and different polymerizable groups. The high-molecular compounds or highly hydrophobic compounds, though being excellent in photosensitizing speed and film strength, may be undesirable in some cases in respect of developing speed and precipitation in the developing solution.

35 The selection and the way to use the addition-polymerizable compound is an important factor for compatibility and dispersibility with other components (e.g. a binder polymer, an initiator, a coloring agent, etc.) contained in the image recording layer. The compatibility may be improved by using e.g. a low-purity compound or a combination of two or more compounds. A specific structure can be selected for the purpose of improving the adhesion of the image recording layer to a substrate, an overcoat layer described later, etc. in the planographic printing plate precursor.

40 In the method of using the polymerizable compound such as compound (C), a suitable structure, compounding and amount of the polymerizable compound can be arbitrarily selected in view of the degree of inhibition of polymeriza-

tion by oxygen, resolution, fogging property, a change in reflectance, and surface adhesiveness. The polymerizable compound can be not only added to the image recording layer, but also constituted as a layer structure or a coating such as an under coating or top coating adjacent to the image recording layer.

Hereinafter, other components in the image recording layer are described in more detail.

<(A) Infrared Absorber>

The image recording layer of the invention contains an infrared absorber having the maximum absorption in a wavelength range of 700 to 1200 nm. By adding the infrared absorber, the planographic printing plate precursor of the invention becomes sensitive to the infrared wavelength range, and can be used for recording by an infrared laser or the like.

In view of compatibility with an easily available high-power laser, it is preferable that the infrared absorber having the maximum absorption in a wavelength range of 700 to 1200 nm is a dye or pigment having the maximum absorption in a wavelength range of 760 to 1200 nm.

As the dye, commercially available dyes and known dyes described in literature, for example, "Senryo Binran (DYE HANDBOOK)" (edited by Organic Synthetic Chemistry Association, issued in 1970) may be utilized. Specific examples of the infrared absorbing dye include azo dyes, metal complex azo dyes, pyrazolone azo dyes, naphthoquinone dyes, anthraquinone dyes, phthalocyanine dyes, carbonium dyes, quinoneimine dyes, methine dyes, cyanine dyes, squalillium dyes, pyrylium salts, metal thiolate complexes, oxonol dyes, diimmonium dyes, aminium dyes and croconium dyes.

Preferable examples of the dye may include cyanine dyes described in JP-A Nos. 58-125246, 59-84356, 59-202829 and 60-78787, methine dyes described in JP-A Nos. 58-173696, 58-181690 and 58-194595, naphthoquinone dyes described in JP-A Nos. 58-112793, 58-224793, 59-48187, 59-73996, 60-52940 and 60-63744, squalillium dyes described in JP-A No. 58-112792 and cyanine dyes described in U.K. Patent No. 434,875.

Near-infrared absorbing sensitizers described in U.S. Pat. No. 5,156,938 are also preferably used. A substituted arylbenzo(thio)pyrylium salt described in U.S. Pat. No. 3,881,459, a trimethinethiapyrylium salt described in JP-A No. 57-142645 (U.S. Pat. No. 4,327,169), pyrylium type compounds described in JP-A Nos. 58-181051, 58-220143, 59-41363, 59-84248, 59-84249, 59-146063 and 59-146061, cyanine dyes described in JP-A No. 59-216146, pentamethinethiopyrylium salts and the like described in U.S. Pat. No. 4,283,475 and pyrylium compounds disclosed in JP-B Nos. 5-13514 and 5-19702 are also preferably used.

Other preferable examples of the infrared absorbing dye may include near-infrared absorbing dyes described as formulae (I) and (II) in U.S. Pat. No. 4,756,993.

Particularly preferable among these dyes are cyanine dyes, phthalocyanine dyes, oxonol dyes, squalylium dyes, pyrylium salts, thiopyrylium dyes, and nickel/thiolate complexes. The dyes represented by formulae (a) to (e) below are preferable because of high light-heat conversion efficiency, among which a cyanine coloring matter represented by formula (a) below is most preferable because when used in the photosensitive composition of the invention, the cyanine coloring matter provides high interaction with alkali-soluble resin and is economical and excellent in stability.



39

and  $R^8$ , which may be the same or different, each independently represent a hydrogen atom or a hydrocarbon group having 12 or less carbon atoms. A hydrogen atom is preferable in view of availability.

$Z_a^-$  represents a counter anion.  $Z_a^-$  is unnecessary when the cyanine dye represented by formula (a) has an anionic substituent in its structure so that charge neutralization is not required. Preferable examples of  $Z_a^-$  are a halogen ion, perchloric acid ion, tetrafluoroborate ion, hexafluorophosphate ion, carboxylic acid ion and sulfonic acid ion in view of the storage stability of the recording layer coating solution. A halogen ion or an organic acid ion such as a carboxylic acid ion or sulfonic acid ion is preferable and a sulfonic acid ion is more preferable and an arylsulfonic acid ion is particularly preferable in view of mutual solubility with an alkali-soluble resin and solubility in the coating solution.

Specific examples of the cyanine dye preferably used in the invention may include, besides those exemplified below, those described in Paragraph Nos. [0017] to [0019] of JP-A No. 2001-133969, Paragraphs No. [0012] to [0038] of JP-A No. 2002-40638 and Paragraph No. [0012] to [0023] of JP-A No. 2002-23360.



40

-continued



41



42



15 In formula (b), L represents a methine chain containing 7 or more conjugated carbon atoms, and the methine chain may have substituent groups, and the substituent groups may be bonded to each other to form a ring structure.  $Z_b^+$  represents a counter cation. The counter cation is preferably 20 ammonium, iodonium, sulfonium, phosphonium, pyridinium and alkali metal cations ( $Ni^+$ ,  $K^+$ ,  $Li^+$ ).  $R^9$  to  $R^{14}$  and  $R^{15}$  to  $R^{20}$  each independently represent a substituent group selected from a hydrogen atom, halogen atom, cyano group, 25 alkyl group, aryl group, alkenyl group, alkynyl group, carbonyl group, thio group, sulfonyl group, sulfinyl group, oxy group and amino group, or a substituent group wherein two or three substituent groups are combined with one another to form a ring structure. The compound of formula 30 (b) wherein L represents a methine chain containing 7 conjugated carbon atoms or all  $R^9$  to  $R^{14}$  and  $R^{15}$  to  $R^{20}$  represent a hydrogen atom, are preferable in view of availability and effect.

35

Examples of the dyes represented by formula (b), which can be used preferably in the invention, include those illustrated below:



-continued



In formula (c),  $Y^3$  and  $Y^4$  each represent an oxygen atom, sulfur atom, selenium atom or tellurium atom;  $M$  represents a methine chain containing 5 or more conjugated carbon atoms;  $R^{21}$  to  $R^{24}$  and  $R^{25}$  to  $R^{28}$  may be the same or different from one another, and represent a hydrogen atom, halogen atom, cyano group, alkyl group, aryl group, alkenyl group, alkynyl group, carbonyl group, thio group, sulfonyl group, sulfinyl group, oxy group or amino group; and  $Z_a^-$  represents a counter anion and has the same meaning as defined for  $Z_a^-$  in formula (a) above.

Examples of the dyes represented by formula (c), which can be used preferably in the invention, include those illustrated below:



Formula (c)

-continued



Formula (d)

In formula (d),  $R^{29}$  to  $R^{31}$  each independently represent a hydrogen atom, alkyl group or aryl group;  $R^{33}$  and  $R^{34}$  each independently represent an alkyl group, a substituted oxy group or a halogen atom;  $n$  and  $m$  each independently represent an integer of 0 to 4;  $R^{29}$  and  $R^{30}$ , or  $R^{31}$  and  $R^{32}$ , may be bonded to each other to form a ring, or  $R^{29}$  and/or  $R^{30}$  may be bonded to  $R^{33}$ , or  $R^{31}$  and/or  $R^{32}$  may be bonded to  $R^{34}$ , to form a ring, and when a plurality of  $R^{33}$  or  $R^{34}$  groups are present,  $R^{33}$  groups or  $R^{34}$  groups may be mutually bonded to form a ring;  $X^2$  and  $X^3$  each independently represent a hydrogen atom, an alkyl group or an aryl group, and at least one of  $X^2$  and  $X^3$  represents a hydrogen atom or an alkyl group;  $Q$  is an optionally substituted trimethine group or pentamethine group which may form a ring structure with a divalent organic group; and  $Z_c^-$  represents a counter anion and is defined as same as  $Z_a^-$  in the above-described formula (a).

Examples of the dyes represented by formula (d), which can be used preferably in the invention, include those illustrated below:



**45**

-continued



Formula (e)

**46**

In formula (e), R<sup>35</sup> to R<sup>50</sup> each independently represent a hydrogen atom, halogen atom, cyano group, alkyl group, aryl group, alkenyl group, alkynyl group, hydroxyl group, carbonyl group, thio group, sulfonyl group, sulfinyl group, oxy group, amino group, and onium salt structure, each of which may have a substituent group; and M represents two hydrogen atoms or a metal atom, halometal group or oxy-metal group. Examples of the metal atom contained therein include the groups IA, IIA, IIIB and IVB atoms in the periodic table, the transition metals in the first, second and third periods, and lanthanoid elements, among which copper, magnesium, iron, zinc, cobalt, aluminum, titanium and vanadium are preferable.

Examples of the dyes represented by formula (e), which can be used preferably in the invention, include those illustrated below:



-continued



Examples of the pigment used as (A) infrared absorber according to the invention include commercially available pigments and pigments described in Color Index (C. I.) Handbook, "Saishin Ganryo Binran (Latest Pigment Handbook)" (edited by Japan Pigment Technology Society, published in 1977), "Saishin Gannryo Oyo Gijyutsu (Latest Pigment Applied Technology)" (CMC Publishing Co., Ltd., published in 1986) and "Insatsu Ink Gijyutsu (Printing Ink Technology)" (CMC Publishing Co., Ltd., published in 1984).

Examples of the type of pigment include black pigments, yellow pigments, orange pigments, brown pigments, red pigments, violet pigments, blue pigments, green pigments, fluorescent pigments, metal powder pigments, and others including polymer bonded dyes. Specifically, as the pigment, insoluble azo pigments, azo lake pigments, condensed azo pigments, chelate azo pigments, phthalocyanine type pigments, anthraquinone type pigments, perylene or perinone type pigments, thioindigo type pigments, quinacridone type pigments, dioxazine type pigments, isoindolone type pigments, quinophthalone type pigments, dyeing lake pigments, azine pigments, nitroso pigments, nitro pigments, natural pigments, fluorescent pigments, inorganic pigments, carbon black may be used. Among these pigments, carbon black is preferable.

These pigments may be used either without being surface-treated or with being surface-treated. As the surface treating methods, a method of coating the surface with a resin or wax, a method of sticking a surfactant and a method of binding a reactive substance (e.g., a silane coupling agent, epoxy compound and polyisocyanate) with the surface of a pigment are considered. The aforementioned surface treating methods are described in "Kinzoku Sekken no Seishitsu to Oyo (Quality and Application of Metal Soaps)" (Saiwai Shobo), "Insatsu Ink Gijyutsu (Printing Ink Technology)"

(CMC Publishing Co., Ltd., published in 1984) and "Saishin Ganryo Oyo Gijyutsu (Latest Pigment Apply Technology)" (CMC Publishing Co., Ltd., published in 1986).

The particle diameter of the pigments is preferably in the range of preferably 0.01 to 10  $\mu\text{m}$ , more preferably 0.05 to 1  $\mu\text{m}$ , and still more preferably 0.1 to 1  $\mu\text{m}$ , in view of the stability of the pigment in the image recording layer coating solution and the uniformity of the image recording layer.

As a method of dispersing the pigment, known dispersing technologies used for the production of ink and toners may be used. Examples of a dispersing machine include a ultrasonic dispersing machine, sand mill, attritor, pearl mill, super mill, ball mill, impeller, disperser, KD mill, colloid mill, dynatron, three-roll mill and pressure kneader. The details of these machines are described in "Saishin Ganryo Oyo Gijyutsu (Latest Pigment Apply Technology)" (CMC Publishing Co., Ltd., published in 1986).

In the invention, one kind of infrared absorber (A) may be used, or two more kinds thereof can also be used.

The infrared absorber (A) in the invention is preferably a cyanine pigment.

In view of sensitivity, the infrared absorber (A) is more preferably a cyanine pigment represented by formula (a), and still more preferably a cyanine pigment represented by formula (a) wherein  $X^1$  is a diarylamino group or  $X^2-L^1$ , and still more preferably the cyanine compound having a diarylamino group.

A cyanine pigment having an electron-withdrawing group or a heavy atom-containing substituent group at each of indolenine sites at both terminals is also preferable, and for example, the one described in Japanese Patent Application No. 2002-278057 is preferably used. A cyanine pigment having an electron-withdrawing group at each of indolenine sites at both terminals, wherein  $X^1$  is a diarylamino group, is most preferable.

Such an infrared absorber may be added to the same layer along with other components, or to a separately provided layer. The infrared absorber is preferably added so that, in the resultant negative-type planographic printing plate precursor, the absorbance of the image recording layer at the maximum absorption at a wavelength in the range of 760 to 1200 nm is in a range of 0.3 to 1.2 in a method of measuring reflection. The absorbance is more preferably in a range of 0.4 to 1.1. In this range, uniform polymerization reaction proceeds in the depth direction of the image recording layer, to provide the film strength of an excellent image region and adhesion to a substrate. The infrared absorber is preferably contained in the image recording layer in an amount of 0.5 to 5% by mass based on the mass of the solid content.

The absorbance of the image recording layer can be regulated by the amount of the infrared absorber added to the image recording layer and the thickness of the image recording layer. The absorbance can be measured in an ordinary manner. Examples of the measurement method include a method wherein the image recording layer whose thickness is determined suitably in a necessary range after drying for the planographic printing plate precursor is formed on a reflective substrate such as aluminum, and then measured for reflection density by an optical densitometer, or a method of measuring density with a spectrophotometer by a reflection method using an integrating sphere.

<(B) Polymerization Initiator>

As the polymerization initiator (B) in the invention, a known radical generating agent can be preferably used. In the invention, the radical generating agent refers to a compound generating radicals by the energy of light and/or heat, to initiate and promote polymerization of a compound having a polymerizable unsaturated group.

As the radical generating agent which can be used in the invention, it is possible to use a known thermally decomposed polymerization initiator, a compound whose bonding dissociation energy is low, a photopolymerization initiator, etc.

Examples of the radical-generating compound include (1) an organic halogenated compound, (2) a carbonyl compound, (3) an organic peroxide compound, (4) an azo polymerization initiator, (5) an azide compound, (6) a metallocene compound, (7) a hexaaryl biimidazole compound, (8) an organic boric acid compound, (9) a disulfonic acid compound, (10) an oxime ester compound and (11) an onium salt compound.

Examples of the organic halogenated compound (1) include compounds described in Wakabayashi et al.: Bull. Chem. Soc. Japan, 42, 2924 (1969), U.S. Pat. No. 3,905,815, JP-B No. 46-4605, JP-A Nos. 48-36281, 55-32070, 60-239736, 61-169835, 61-169837, 62-58241, 62-212401, 63-70243, 63-298339, and M. P. Hutt: Journal of Heterocyclic Chemistry, 1 (No. 3), (1970), particularly oxazole compounds substituted with a trihalomethyl group (S-triazine compounds).

The organic halogenated compound (1) is more preferably an S-triazine derivative wherein at least one mono, di or trihalogen-substituted methyl group is bonded to an S-triazine ring, and specific examples include 2,4,6-tris(monochloromethyl)-S-triazine, 2,4,6-tris(dichloromethyl)-S-triazine, 2,4,6-tris(trichloromethyl)-S-triazine, 2-methyl-4,6-bis(trichloromethyl)-S-triazine, 2-n-propyl-4,6-bis(trichloromethyl)-S-triazine, 2-( $\alpha$ , $\alpha$ , $\beta$ -trichloroethyl)-4,6-bis(trichloromethyl)-S-triazine, 2-phenyl-4,6-bis(trichloromethyl)-S-triazine, 2-(p-methoxyphenyl)-4,6-bis(trichloromethyl)-S-triazine, 2-(3,4-epoxyphenyl)-4,6-bis(trichloromethyl)-S-triazine,

triazine, 2-(p-chlorophenyl)-4,6-bis(trichloromethyl)-S-triazine, 2-[1-(p-methoxyphenyl)-2,4-butadienyl]-4,6-bis(trichloromethyl)-S-triazine, 2-styryl-4,6-bis(trichloromethyl)-S-triazine, 2-(p-methoxystyryl)-4,6-bis(trichloromethyl)-S-triazine, 2-(p-1-propyloxystyryl)-4,6-bis(trichloromethyl)-S-triazine, 2-(p-tolyl)-4,6-bis(trichloromethyl)-S-triazine, 2-(4-naphthoxynaphthyl)-4,6-bis(trichloromethyl)-S-triazine, 2-phenylthio-4,6-bis(trichloromethyl)-S-triazine, 2-benzylthio-4,6-bis(trichloromethyl)-S-triazine, 2,4,6-tris(dibromomethyl)-S-triazine, 2,4,6-tris(tribromomethyl)-S-triazine, 2-methyl-4,6-bis(tribromomethyl)-S-triazine, 2-methoxy-4,6-bis(tribromomethyl)-S-triazine, etc.

Examples of the carbonyl compound (2) include benzophenone, benzophenone derivatives such as Michler's ketone, 2-methyl benzophenone, 3-methyl benzophenone, 4-methyl benzophenone, 2-chlorobenzophenone, 4-bromobenzophenone, 2-carboxybenzophenone, etc., acetophenone derivatives such as 2,2-dimethoxy-2-phenyl acetophenone, 2,2-diethoxy acetophenone, 1-hydroxycyclohexylphenyl ketone,  $\alpha$ -hydroxy-2-methyl phenyl propane, 1-hydroxy-1-methylethyl-(p-isopropylphenyl) ketone, 1-hydroxy-1-(p-dodecylphenyl) ketone, 2-methyl-(4'-methylthio) phenyl-2-morpholino-1-propanone, 1,1,1-trichloromethyl-(p-butylphenyl) ketone, etc., thioxanthone, thioxanthone derivatives such as 2-ethyl thioxanthone, 2-isopropyl thioxanthone, 2-chlorothioxanthone, 2,4-dimethyl thioxanthone, 2,4-diethyl thioxanthone, 2,4-diisopropyl thioxanthone, etc., and benzoate esters such as ethyl p-dimethylaminobenzoate, ethyl p-diethylaminobenzoate, etc.

Examples of the organic peroxide compound (3) include trimethyl cyclohexanone peroxide, acetyl acetone peroxide, 1,1-bis(tert-butylperoxy)-3,3,5-trimethyl cyclohexane, 1,1-bis(tert-butylperoxy) cyclohexane, 2,2-bis(tert-butylperoxy) butane, tert-butyl hydroperoxide, cumene hydroperoxide, diisopropyl benzene hydroperoxide, 2,5-dimethylhexane-2,5-dihydroperoxide, 1,1,3,3-tetramethyl butyl hydroperoxide, tert-butyl cumyl peroxide, dicumyl peroxide, 2,5-dimethyl-2,5-di(tert-butylperoxy) hexane, 2,5-oxanoyl peroxide, succinate peroxide, benzoyl peroxide, 2,4-dichlorobenzoyl peroxide, diisopropyl peroxy dicarbonate, di-2-ethylhexyl peroxy dicarbonate, di-2-ethoxyethyl peroxy dicarbonate, dimethoxy isopropyl peroxy carbonate, di-(3-methyl-3-methoxybutyl) peroxy dicarbonate, tert-butyl peroxy acetate, tert-butyl peroxy pivalate, tert-butyl peroxy neodecanoate, tert-butyl peroxy octanoate, tert-butyl peroxy laurate, tertiary carbonate, 3,3',4,4'-tetra-(t-butylperoxycarbonyl) benzophenone, 3,3',4,4'-tetra-(t-hexylperoxycarbonyl) benzophenone, 3,3',4,4'-tetra-(p-isopropylcumylperoxycarbonyl) benzophenone, carbonyl di(t-butylperoxy dihydrogen diphthalate), carbonyl di(t-hexylperoxy dihydrogen diphthalate), etc.

As the azo polymerization initiator (4), azo compounds described in, for example, JP-A No. 8-108621 can be used.

Examples of the metallocene compound (6) include various titanocene compounds described in JP-A Nos. 59-152396, 61-151197, 63-41484, 2-249, 2-4705 and 5-83588, for example, di-cyclopentadienyl-Ti-bis-phenyl, di-cyclopentadienyl-Ti-bis-2,6-difluorophen-1-yl, di-cyclopentadienyl-Ti-bis-2,4,6-trifluorophen-1-yl, di-cyclopentadienyl-Ti-bis-2,3,5,6-tetrafluorophen-1-yl, di-cyclopentadienyl-Ti-bis-2,3,4,5,6-cyclopentafluorophen-1-yl, di-methylcyclopentadienyl-Ti-bis-2,6-difluorophen-1-yl, di-methylcyclopentadienyl-Ti-bis-2,4,6-trifluorophen-1-yl, di-methylcyclopentadienyl-Ti-bis-2,3,5,6-tetrafluorophen-

51

1-yl, di-methylcyclopentadienyl-Ti-bis-2,3,4,5,6-pentafluorophen-1-yl, and iron-allene complexes described in JP-A Nos. 1-304453 and 1-152109.

Examples of the hexaaryl biimidazole compound (7) include various compounds described in JP-B 6-29285, U.S. Pat. Nos. 3,479,185, 4,311,783, and 4,622,286, specifically 2,2'-bis(o-chlorophenyl)-4,4',5,5'-tetraphenyl biimidazole, 2,2'-bis(o-bromophenyl)-4,4',5,5'-tetraphenyl biimidazole, 2,2'-bis(o,p-dichlorophenyl)-4,4',5,5'-tetraphenyl biimidazole, 2,2'-bis(o-chlorophenyl)-4,4',5,5'-tetra(m-methoxyphenyl) biimidazole, 2,2'-bis(o,o'-dichlorophenyl)-4,4',5,5'-tetraphenyl biimidazole, 2,2'-bis(o-nitrophenyl)-4,4',5,5'-tetraphenyl biimidazole, 2,2'-bis(o-methylphenyl)-4,4',5,5'-tetraphenyl biimidazole, 2,2'-bis(o-trifluorophenyl)-4,4',5,5'-tetraphenyl biimidazole, etc.

Examples of the organic borate compound (8) include organic borate compounds described in JP-A Nos. 62-143044, 62-150242, 9-188685, 9-188686, 9-188710, 2000-131837, 2002-107916, Japanese Patent No. 2764769, JP-A No. 2002-116539, and Kunz, Martin: Rad Tech '98, Proceeding Apr. 19-22, 1998, Chicago, organic boron sulfonium complexes or organic boron oxosulfonium complexes described in JP-A Nos. 6-157623, 6-175564 and 6-175561, organic boron iodonium complexes described in JP-A Nos. 6-175554 and 6-175553, organic phosphonium complexes described in JP-A No. 9-188710, and organic boron transition metal coordination complexes described in JP-A Nos. 6-348011, 7-128785, 7-140589, 7-306527 and 7-292014.

Examples of the disulfone compound (9) include compounds described in JP-A Nos. 61-166544 and 2002-328465.

Examples of the oxime ester compound (10) include compounds described in J. C. S. Perkin II (1979) 1653-1660, J. C. S. Perkin II (1979) 156-162, Journal of Photopolymer Science and Technology (1995) 202-232 and JP-A No. 2000-66385 and compounds described in JP-A No. 2000-80068, specifically the following compounds:

52

-continued



**53**

-continued

**54**

-continued



-continued



Examples of the onium salt compound (11) include diazonium salts described in S. I. Schlesinger, Photogr. Sci. Eng., 18, 387 (1974) and T. S. Bal et al., Polymer, 21, 423 (1980), ammonium salts described in U.S. Pat. No. 4,069,055 and JP-A No. 4-365049, phosphonium salts described in U.S. Pat. Nos. 4,069,055 and 4,069,056, iodonium salts described in European Patent No. 104,143, U.S. Pat. Nos. 339,049 and 410,201, JP-A Nos. 2-150848 and 2-296514, sulfonium salts described in European Patent Nos. 370,693, 390, 214, 233, 567, 297,443 and 297,442, U.S. Pat. Nos. 4,933,377, 161,811, 410,201, 339,049, 4,760,013, 4,734,444 and 2,833,827, and German Patent Nos. 2,904,626, 3,604, 580 and 3,604,581, selenium salts described in J. V. Crivello et al., Macromolecules, 10(6), 1307 (1977) and J. V. Crivello

et al., J. Polymer Sci., Polymer Chem. Ed., 17, 1047 (1979), onium salts such as arsonium salts described in C. S. Wen et al., Teh, Proc. Conf. Rad. Curing ASIA, p. 478, Tokyo, October (1988), etc.

5 Particularly, the oxime ester compound (10) or the onium salt compound (11) such as a diazonium salt, iodonium salt and sulfonium salt can be mentioned in respect of reactivity and stability. In the invention, these onium salts function not as acid generating agents but as ionic radical polymerization initiators.

The onium salts used preferably in the invention are onium salts represented by formulae (RI-I) to (RI-III):



In formula (RI-I),  $\text{Ar}^1$  represents an aryl group containing 20 or less carbon atoms, which may have 1 to 6 substituent groups, and the substituent group is preferably an alkyl group containing 1 to 12 carbon atoms, an alkenyl group containing 1 to 12 carbon atoms, an alkynyl group containing 1 to 12 carbon atoms, an aryl group containing 1 to 12 carbon atoms, an alkoxy group containing 1 to 12 carbon atoms, an aryloxy group containing 1 to 12 carbon atoms, a halogen atom, an alkylamino group containing 1 to 12 carbon atoms, a dialkylamino group containing 1 to 12 carbon atoms, an alkyl amide group or aryl amide group containing 1 to 12 carbon atoms, a carbonyl group, a carboxyl group, a cyano group, a sulfonyl group, a thioalkyl group containing 1 to 12 carbon atoms and a thioaryl group containing 1 to 12 carbon atoms.  $(\text{Z}^{11})^-$  represents a monovalent anion including a halogen ion, perchlorate ion, hexafluorophosphate ion, tetrafluoroborate ion, sulfonate ion, sulfinate ion, thiosulfonate ion and sulfate ion, and a perchlorate ion, hexafluorophosphate ion, tetrafluoroborate ion, sulfonate ion and sulfinate ion are preferable in view of safety.

50 In formula (RI-II),  $\text{Ar}^{11}$  and  $\text{Ar}^{22}$  each independently represent an aryl group containing 20 or less carbon atoms, which may have 1 to 6 substituent groups, and the substituent group is preferably an alkyl group containing 1 to 12 carbon atoms, an alkenyl group containing 1 to 12 carbon atoms, an alkynyl group containing 1 to 12 carbon atoms, an aryl group containing 1 to 12 carbon atoms, an alkoxy group containing 1 to 12 carbon atoms, an aryloxy group containing 1 to 12 carbon atoms, a halogen atom, an alkylamino group containing 1 to 12 carbon atoms, a dialkylamino group containing 1 to 12 carbon atoms, an alkyl amide group or aryl amide group containing 1 to 12 carbon atoms, a carbonyl group, a carboxyl group, a cyano group, a sulfonyl group, a thioalkyl group containing 1 to 12 carbon atoms and a thioaryl group containing 1 to 12 carbon atoms. ( $\text{Z}^{21}$ )

55 60 65 represents a monovalent anion including a halogen ion, perchlorate ion, hexafluorophosphate ion, tetrafluoroborate ion, sulfonate ion, sulfinate ion, thiosulfonate ion and sulfate

57

ion, and a perchlorate ion, hexafluorophosphate ion, tetrafluoroborate ion, sulfonate ion, sulfinate ion and carboxylate ion are preferable in view of safety and reactivity.

In formula (RI-III), R<sup>31</sup>, R<sup>32</sup> and R<sup>33</sup> each independently represent an aryl group, alkyl group, alkenyl group or alkynyl group containing 20 or less carbon atoms which may have 1 to 6 substituent groups, and is preferably an aryl group in respect of reactivity and safety. The substituent group is preferably an alkyl group containing 1 to 12 carbon atoms, an alkenyl group containing 1 to 12 carbon atoms, an alkynyl group containing 1 to 12 carbon atoms, an aryl group containing 1 to 12 carbon atoms, an alkoxy group containing 1 to 12 carbon atoms, an aryloxy group containing 1 to 12 carbon atoms, a halogen atom, an alkylamino group containing 1 to 12 carbon atoms, a dialkylamino group containing 1 to 12 carbon atoms, an alkyl amide group or aryl amide group containing 1 to 12 carbon atoms, a carbonyl group, a carboxyl group, a cyano group, a sulfonyl group, a thioalkyl group containing 1 to 12 carbon atoms and a thioaryl group containing 1 to 12 carbon atoms. (Z<sup>31</sup>)<sup>-</sup> represents a monovalent anion including a halogen ion, perchlorate ion, hexafluorophosphate ion, tetrafluoroborate ion, sulfonate ion, sulfinate ion, thiosulfonate ion and sulfate ion, and a perchlorate ion, hexafluorophosphate ion, tetrafluoroborate ion, sulfonate ion, sulfinate ion and carboxylate ion are preferable in view of safety and reactivity, and (Z<sup>31</sup>)<sup>-</sup> is particularly preferably a carboxylate ion in JP-A No. 2001-343742, and still more preferably a carboxylate ion in JP-A No. 2002-148790.

The onium salt compounds serving as the polymerization initiator usable preferably in the invention include, but are not limited, to the following examples:



(N-1)

40



(N-2)

50



(N-3)

55



(N-4)

60

ClO<sub>4</sub><sup>-</sup>

65

58

-continued



(N-5)

BF<sub>4</sub><sup>-</sup>

(N-6)



(N-7)



(N-8)

ClO<sub>4</sub><sup>-</sup>

(N-9)



(N-10)



(N-11)

PF<sub>6</sub><sup>-</sup>

65

59

-continued



60

-continued

(I-8)



**61**

-continued



PF6-

ClO4-



CF3SO3-

**62**

-continued

5

(S-1)



10

(S-2)



15

(S-3)



20

(S-4)

25

(S-5)



30

(S-6)

35

(S-7)



40

(S-8)

45

(S-9)



50

(S-10)



55

(S-11)



(S-12)

(S-13)

(S-14)

(S-15)

(S-16)

(S-17)

(S-18)

The polymerization initiator (B) may be added in the image recording layer preferably in an amount of 0.1 to 50% by mass, more preferably 0.5 to 30% by mass, and still more preferably 1 to 20% by mass, based on the mass of the solid content of the image recording layer. In this range, good sensitivity and excellent stain resistance of a non-image region during printing can be achieved. These polymerization initiators may be used alone or as a mixture of two or more thereof. The polymerization initiator, along with other components, may be added to the same layer or to a separately provided layer.

In addition to the essential components described above, various compounds may be added to the image recording layer of the invention in accordance with the purpose.

<(D) Binder Polymer>

In view of improving layer-forming properties, the binder polymer (D) is added preferably to the image recording layer of the invention. As the binder polymer which can be used in the invention, a conventionally known binder polymer can be used without limitation, and a film-forming linear organic polymer is preferable. Examples of such binder polymers include acrylic resin, polyvinyl acetal resin, polyurethane resin, polyurea resin, polyimide resin, polyamide resin, epoxy resin, methacrylic resin, polystyrene resin, novolak phenol resin, polyester resin, synthetic rubber and natural rubber.

To improve the strength of a film in an image region, the binder polymer preferably has crosslinkability. To allow the binder polymer to have crosslinkability, crosslinking functional groups such as ethylenically unsaturated bonds may be introduced into a main chain or side chain of the polymer. The crosslinking functional groups may be introduced by copolymerization.

Examples of the polymer having an ethylenically unsaturated bond in a main chain of the molecule include poly-1,4-butadiene, poly-1,4-isoprene, etc.

Examples of the polymer having an ethylenically unsaturated bond in a side chain of the molecule include a polymer of an ester or amide of acrylic acid or methacrylic acid wherein the ester or amide residue (R in —COOR or —CONHR) has an ethylenically unsaturated bond.

Examples of the residue (the above-mentioned R) having an ethylenically unsaturated bond include  $-(CH_2)_nCR^1=CR^2R^3$ ,  $-(CH_2O)_nCH_2CR^1=CR^2R^3$ ,  $-(CH_2CH_2O)_nCH_2CR^1=CR^2R^3$ ,  $-(CH_2)_nNH-CO-O-CH_2CR^1=CR^2R^3$ ,  $-(CH_2)_nO-CO-CR^1=CR^2R^3$  and  $-(CH_2CH_2O)_n-X$  wherein R<sup>1</sup> to R each independently represent a hydrogen atom, a halogen atom or an alkyl, aryl, alkoxy or aryloxy group having 1 to 20 carbon atoms, R<sup>1</sup> and R<sup>2</sup> or R<sup>3</sup> may be bonded to each other to form a ring, n is an integer of 1 to 10, and X represents a dicyclopentadienyl residue.

Examples of the ester residue include  $-CH_2CH=CH_2$  (described in JP-B 7-21633),  $-CH_2CH_2O-CH_2CH=CH_2$ ,  $-CH_2C(CH_3)=CH_2$ ,  $-CH_2CH=CH-C_6H_5$ ,  $-CH_2CH_2OCOCH=CH-C_6H_5$ ,  $-CH_2CH_2-NHCOO-CH_2CH=CH_2$ , and  $-CH_2CH_2O-X$  wherein X represents a dicyclopentadienyl residue.

Examples of the amide residue include  $-CH_2CH=CH_2$ ,  $-CH_2CH_2-Y$  (Y is a cyclohexene residue) and  $-CH_2CH_2-OCO-CH=CH_2$ .

The crosslinking binder polymer is cured, for example, by adding a free radical (a polymerization initiation radical or a growing radical in a process of polymerizing a polymerizable compound) to its crosslinking functional group, thereby initiating addition polymerization directly among

the polymers or via polymerizing linkage of the polymerizable compound, to form crosslinkages between polymer molecules. Alternatively, an atom (for example, a hydrogen atom in a carbon atom adjacent to the functional crosslinking group) in the polymer is withdrawn by a free radical to generate polymer radicals, which are then bonded to one another to form crosslinkages among polymer molecules, whereby the binder polymer is cured.

The content of the crosslinking group in the binder polymer (content of radical-polymerizable unsaturated double bonds determined by iodine titration) is preferably 0.1 to 10.0 mmol, more preferably 1.0 to 7.0 mmol, and most preferably 2.0 to 5.5 mmol, per g of the binder polymer. In this range, good sensitivity and good shelf stability can be achieved.

In view of improving the in-machine development properties of a region not exposed to light in the image recording layer, the binder polymer is preferably a compound having high solubility or dispersibility in ink and/or dampening water.

For improving solubility or dispersibility in ink, the binder polymer is preferably lipophilic, and for improving solubility or dispersibility in dampening water, the binder polymer is preferably hydrophilic. Accordingly, simultaneous use of a lipophilic binder polymer and a hydrophilic binder polymer is also effective in the invention.

The hydrophilic binder is preferably the one having a hydrophilic group such as, for example, a hydroxy group, carboxyl group, carboxylate group, hydroxyethyl group, polyoxyethyl group, hydroxypropyl group, polyoxypropyl group, amino group, aminoethyl group, aminopropyl group, ammonium group, amide group, carboxymethyl group, sulfonate group and phosphate group.

Specific examples of the hydrophilic binder polymer include gum arabic, casein, gelatin, starch derivatives, carboxymethyl cellulose and sodium salts thereof, cellulose acetate, sodium alginate, vinyl acetate-maleic acid copolymers, styrene-maleic acid copolymers, polyacrylic acids and salts thereof, polymethacrylic acids and salts thereof, hydroxyethyl methacrylate homopolymers and copolymers, hydroxyethyl acrylate homopolymers and copolymers, hydroxypropyl methacrylate homopolymers and copolymers, hydroxypropyl acrylate homopolymers and copolymers, hydroxybutyl methacrylate homopolymers and copolymers, hydroxybutyl acrylate homopolymers and copolymers, polyethylene glycols, hydroxypropylene polymers, polyvinyl alcohols, polyvinyl acetate hydrolyzed at least 60% by weight, preferably at least 80% by weight, polyvinyl formal, polyvinyl butyral, polyvinyl pyrrolidone, acrylamide homopolymers and copolymers, methacrylamide homopolymers and copolymers, N-methylol acrylamide homopolymers and copolymers, polyvinyl pyrrolidone, alcohol-soluble nylon, 2,2-bis-(4-hydroxyphenyl)-propane/epichlorohydrin polyether, etc.

The weight-average molecular weight of the binder polymer (D) is preferably 5,000 or more, and more preferably in the range of 10,000 to 300,000. The number-average molecular weight thereof is preferably 1,000 or more, and more preferably in the range of 2,000 to 250,000. Polydispersity (weight-average molecular weight/number-average molecular weight) is preferably in the range of 1.1 to 10.

The binder polymer (D) may be a random polymer, block polymer or graft polymer, preferably a random polymer.

The binder polymer (D) can be synthesized in a method known in the art. Examples of the solvent used in synthesis include tetrahydrofuran, ethylene dichloride, cyclohexanone, methyl ethyl ketone, acetone, methanol, ethanol,

ethylene glycol monomethyl ether, ethylene glycol monoethyl ether, 2-methoxyethyl acetate, diethylene glycol dimethyl ether, 1-methoxy-2-propanol, 1-methoxy-2-propyl acetate, N,N-dimethyl formamide, N,N-dimethyl acetamide, toluene, ethyl acetate, methyl lactate, ethyl lactate, dimethyl sulfoxide, and water. These solvents are used alone or as a mixture thereof.

As the radical polymerization initiator used for synthesizing the binder polymer (D), known compounds such as an azo-type initiator or a peroxide initiator can be used.

The binder polymers (D) may be used alone or as a mixture of one or more thereof.

The binder polymer (D) may be contained in the image recording layer preferably in an amount of 10 to 90% by mass, more preferably 20 to 80% by mass, and still more preferably 30 to 70% by mass, based on the mass of the total solid content of the image recording layer. In this range, good strength of an image region and image formability can be achieved.

The polymerizable compound represented by (C) and the binder polymer (D) are used preferably in a ratio of from 1/9 to 7/3 by weight.

#### <(F) Microcapsule>

Preferably, the image forming layer of the invention further comprises microcapsules. By the presence of microcapsules, microcapsule wall materials in a region exposed to light are melted in a light-exposed region to adhere to a substrate, or adjacent microcapsules with their softened surface are fused with one another and adhere to the surface of the substrate to easily form a hydrophobic region thereon, and even if microcapsules in a region not exposed to light are dispersed in a hydrophilic binder, the microcapsules together with the binder are easily removed with a small amount of water, thus improving image formability. Such microcapsules may be added as fillers, and may have incorporated the image recording layer constituent components (A) to (D) and other constituent components described later.

In the invention, some modes can be used in a method of incorporating the image recording layer constituent components (A) to (D) and at least one of other constituent components described later into the image recording layer. One mode is a molecule-dispersed image recording layer to be applied by dissolving the constituent components in a suitable solvent as described in JP-A No. 2002-287334. Another mode is a microcapsule-type image recording layer wherein the whole or a part of the constituent components are incorporated into microcapsules to be contained in the image recording layer as described in JP-A Nos. 2001-277740 and 2001-277742. In the microcapsule-type image recording layer, the constituent components may also be contained in material other than microcapsules. In a preferable mode of the microcapsule-type image recording layer, the hydrophobic constituent components are contained in microcapsules, while the hydrophilic constituent components are contained in material other than microcapsules. For attaining higher in-machine development properties, the image recording layer is preferably a microcapsule-type image recording layer.

For producing microcapsules of the image-recording layer constituent components (A) to (D), conventional methods can be used. Examples of the method of producing microcapsules include, but are not limited to, a method of utilizing coacervation as shown in U.S. Pat. Nos. 2,800,457 and 2,800,458, a method of interfacial polymerization as shown in U.S. Pat. No. 3,287,154, JP-B 38-19574 and JP-B 42-446, a method of precipitating polymers as shown in U.S.

Pat. Nos. 3,418,250 and 3,660,304, a method of using an isocyanate polyol wall material as shown in U.S. Pat. No. 3,796,669, a method of using an isocyanate wall material as shown in U.S. Pat. No. 3,914,511, a method of using an urea-formaldehyde type or urea-formaldehyde-resorcinol type wall-forming material as shown in U.S. Pat. Nos. 4,001,140, 4,087,376 and 4,089,802, a method of using a wall material such as melamine-formaldehyde resin and hydroxy cellulose as shown in U.S. Pat. No. 4,025,445, a method of in situ polymerization of monomers as shown in JP-B 36-9163 and JP-B 51-9079, a method of spray drying as shown in GB Patent No. 930422 and U.S. Pat. No. 3,111,407, and a method of electrolytic dispersion cooling as shown in GB Patent Nos. 952807 and 967074.

15 The microcapsule wall used in the invention preferably has 3-dimensional crosslinkages to be swollen with a solvent. In this respect, the wall material for the microcapsules is preferably polyurea, polyurethane, polyester, polycarbonate, polyamide and a mixture thereof, among which polyurea and polyurethane are particularly preferable. A compound having a crosslinking functional group such as an ethylenically unsaturated bond capable of being introduced into the binder polymer (D) may be introduced into the microcapsule wall.

20 The average particle diameter of the microcapsules is preferably 0.01 to 3.0  $\mu\text{m}$ , more preferably 0.05 to 2.0  $\mu\text{m}$  and most preferably 0.10 to 1.0  $\mu\text{m}$ . In this range, excellent resolution and storability can be achieved.

#### <Surfactant>

25 In the invention, a surfactant is used preferably in the image recording layer in order to promote in-machine development properties upon initiation of printing and to improve the state of a coating surface. Examples of the surfactant include a nonionic surfactant, anionic surfactant, cationic surfactant, amphoteric surfactant and fluorine-based surfactant. The surfactants may be used alone or as a mixture of two or more thereof.

30 The nonionic surfactant used in the invention is not particularly limited, and a conventionally known nonionic surfactant can be used. Examples include polyoxyethylene alkyl ethers, polyoxyethylene alkyl phenyl ethers, polyoxyethylene polystyryl phenyl ethers, polyoxyethylene polyoxypropylene alkyl ethers, glycerin fatty partial esters, sorbitan fatty partial esters, pentaerythritol fatty partial esters, propylene glycol monofatty esters, sucrose fatty partial esters, polyoxyethylene sorbitan fatty partial esters, polyoxyethylene sorbitol fatty partial esters, polyethylene glycol fatty esters, polyglycerin fatty partial esters, polyoxyethylene castor oil, polyoxyethylene glycerin fatty partial esters, fatty acid diethanol amides, N,N-bis-2-hydroxyalkyl amines, polyoxyethylene alkyl amine, triethanol amine fatty ester, trialkyl amine oxide, polyethylene glycol, and a polyethylene glycol/polypropylene glycol copolymer.

35 The anionic surfactant used in the invention is not particularly limited, and a conventionally known anionic surfactant can be used. Examples include aliphatic acid salts, abietates, hydroxylkane sulfonates, alkane sulfonates, dialkylsulfosuccinates, linear alkyl benzene sulfonates, branched alkyl benzene sulfonates, alkyl naphthalene sulfonates, alkyl phenoxy polyoxyethylene propyl sulfonates, polyoxyethylene alkyl sulfophenyl ether salts, N-methyl-N-oleyl taurine sodium salt, N-alkyl sulfosuccinic monoamide disodium salt, petroleum sulfonates, sulfuric tallow oil, fatty alkyl ester sulfates, alkyl sulfates, polyoxyethylene alkyl ether sulfates, fatty monoglyceride sulfates, polyoxyethylene alkyl phenyl ether sulfates, polyoxyethylene styryl phe-

nyl ether sulfates, alkyl phosphates, polyoxyethylene alkyl ether phosphates, polyoxyethylene alkyl phenyl ether phosphates, partially saponified styrene/maleic anhydride copolymers, partially saponified olefin/maleic anhydride copolymers and naphthalene sulfonate formalin condensates.

The cationic surfactant used in the invention is not particularly limited, and a conventionally known cationic surfactant can be used. Examples include alkyl amine salts, quaternary ammonium salts, polyoxyethylene alkyl amine salts and polyethylene polyamine derivatives.

The amphoteric surfactant used in the invention is not particularly limited, and a conventionally known amphoteric surfactant can be used. Examples include carboxy betaines, aminocarboxylic acids, sulfobetaines, aminosulfates and imidazolines.

The term "polyoxyethylene" in the surfactants described above can be read as "polyoxyalkylene" such as polyoxymethylene, polyoxypropylene, polyoxybutylene, etc., and their surfactants can also be used in the invention.

Further preferable surfactants are fluorine-based surfactants containing a perfluoroalkyl group in their molecule. Such fluorine-based surfactants include anionic surfactants such as perfluoroalkyl carboxylates, perfluoroalkyl sulfonates and perfluoroalkyl phosphates, amphoteric surfactants such as perfluoroalkyl betaine, cationic surfactants such as perfluoroalkyl trimethyl ammonium salts, and non-ionic surfactants such as perfluoroalkyl amine oxide, perfluoroalkyl ethylene oxide adducts, perfluoroalkyl group- and hydrophilic group-containing oligomers, perfluoroalkyl group- and lipophilic group-containing oligomers, perfluoroalkyl group-, hydrophilic group- and lipophilic group-containing oligomers, and perfluoroalkyl group- and lipophilic group-containing urethane. Preferable examples also include fluorine-based surfactants described in JP-A Nos. 62-170950, 62-226143 and 60-1.68144.

The surfactants can be used alone or as a mixture of two or more thereof.

The surfactant may be contained in the image recording layer preferably in an amount of 0.001 to 10% by mass, and more preferably 0.01 to 5% by mass, based on the mass of the total solid content of the image recording layer.

#### <Coloring Agent>

In the invention, various compounds other than the above-mentioned compounds may be added if necessary. For example, dyes having large absorption in the visible light range can be used as coloring agents of images. Specific examples include Oil Yellow #101, Oil Yellow #103, Oil Pink #312, Oil Green BG, Oil Blue BOS, Oil Blue #603, Oil Black BY, Oil Black BS, Oil Black T-505 (which are available from Orient Chemical Industries, Ltd.), Victoria Pure Blue, Crystal Violet (CI42555), Methyl Violet (CI42535), Ethyl Violet, Rhodamine B (CI145170B), Malachite Green (CI42000), Methylene Blue (CI52015), and dyes described in JP-A No. 62-293247. Pigments such as phthalocyanine pigment, azo pigment, carbon black and titanium oxide can also be preferably used.

Such a coloring agent is preferably added to the image recording layer in order to distinguish the image region from the non-image region after image formation. The coloring agent is preferably contained in the image recording layer in an amount of 0.01 to 10% by mass based on the mass of the total solid content of the image recording layer.

#### <Printing-Out Agent>

A compound discoloring with an acid or radical for forming an image printed out can be added to the image

recording layer of the invention. Examples of such compound include various coloring matters based on diphenyl methane, triphenyl methane, thiazine, oxazine, xanthene, anthraquinone, iminoquinone, azo, azomethine, etc.

Specific examples include dyes such as Brilliant Green, Ethyl Violet, Methyl Green, Crystal Violet, Basic Fuchsin, Methyl Violet 2B, Quinaldine Red, Rose Bengal, Metanil Yellow, Thymol Sulfophthalein, Xylenol Blue, Methyl Orange, Paramethyl Red, Congo Red, Benzopurpurine 4B,  $\alpha$ -Naphthyl Red, Nile Blue 2B, Nile Blue A, Methyl Violet, Malachite Green, Parafuchsin, Victoria Pure Blue BOH [manufactured by Hodogaya Kagaku Co., Ltd.], Oil Blue #603 [manufactured by Orient Chemical Industries, Ltd.], Oil Pink #312 [manufactured by Orient Chemical Industries, Ltd.], Oil Red 5B [manufactured by Orient Chemical Industries, Ltd.], Oil Scarlet #308. [manufactured by Orient Chemical Industries, Ltd.], Oil Red OG [manufactured by Orient Chemical Industries, Ltd.], Oil Red RR [manufactured by Orient Chemical Industries, Ltd.], Oil Green #502 [manufactured by Orient Chemical Industries, Ltd.], Spirone Red BEH Special [manufactured by Hodogaya Kagaku Co., Ltd.], m-Cresol Purple, Cresol Red, Rhodamine B, Rhodamine 6G, Sulforhodamine B, Auramine, 4-p-diethylaminophenyl iminonaphthoquinone, 2-carboxyanilino-4-p-diethylaminophenyl iminonaphthoquinone, 2-carboxy-3-tearylamino-4-p-N,N-bis(hydroxyethyl) amino-phenyliminonaphthoquinone, 1-phenyl-3-methyl-4-p-diethylaminophenylimino-5-pyrazolone and 1-P-naphthyl-4-p-diethylaminophenylimino-5-pyrazolone, and leuco dyes such as p,p',p"-hexamethyl triaminophenyl methane (Leuco Crystal Violet) and Pergascript Blue SRB (manufactured by Ciba-Geigy).

In addition to those described above, preferable examples include leuco dyes known as material of thermal sensitive paper and pressure sensitive paper. Specific examples include crystal violet lactone, malachite green lactone, benzoyl leucomethylene blue, 2-(N-phenyl-N-methylamino)-6-(N-p-tolyl-N-ethyl) amino-fluoran, 2-anilino-3-methyl-6-(N-ethyl-p-toluidino) fluoran, 3,6-dimethoxy fluoran, 3-(N,N-diethylamino)-5-methyl-7-(N,N-dibenzylamino)-fluoran, 3-(N-cyclohexyl-N-methylamino)-6-methyl-7-anilinofluoran, 3-(N,N-diethylamino)-6-methyl-7-anilinofluoran, 3-(N,N-diethylamino)-6-methyl-7-xylidinofluoran, 3-(N,N-diethylamino)-6-methyl-7-chlorofluoran, 3-(N,N-diethylamino)-6-methoxy-7-aminofluoran, 3-(N,N-diethylamino)-7-(4-chloroanilino) fluoran, 3-(N,N-diethylamino)-7-chlorofluoran, 3-(N,N-diethylamino)-7-benzyl aminofluoran, 3-(N,N-diethylamino)-7,8-benzofluoran, 3-(N,N-dibutylamino)-6-methyl-7-anilinofluoran, 3-(N,N-dibutylamino)-6-methyl-7-xylidinofluoran, 3-piperidino-6-methyl-7-anilinofluoran, 3-pyrrolidino-6-methyl-7-anilinofluoran, 3,3-bis(1-ethyl-2-methylindol-3-yl) phthalide, 3,3-bis(1-n-butyl-2-methylindol-3-yl) phthalide, 3,3-bis(p-dimethylaminophenyl)-6-dimethyl amino phthalide, 3-(4-diethylamino-2-ethoxyphenyl)-3-(1-ethyl-2-methylindol-3-yl)-4-zaphthalide, 3-(4-diethylaminophenyl)-3-(1-ethyl-2-methylindol-3-yl) phthalide, etc.

The dye that is discolored due to acid or radical is contained in the image recording layer in an amount of 0.01 to 10% by mass based on the mass of the solid content of the image recording layer.

#### <Polymerization Inhibitor>

A small amount of a heat-polymerization inhibitor is preferably added to the image recording layer of the invention in order to inhibit undesired heat polymerization of the

radical polymerizable compound (C) during the production or storage of the image recording layer.

Preferable examples of the heat-polymerization inhibitor include hydroquinone, p-methoxyphenol, di-t-butyl-p-cresol, pyrogallol, t-butyl catechol, benzoquinone, 4,4'-thio-bis(3-methyl-6-t-butyl phenol), 2,2'-methylene bis(4-methyl-6-t-butyl phenol), N-nitroso-N-phenyl hydroxylamine aluminum salt, etc.

The heat-polymerization inhibitor is preferably contained in the image recording layer in an amount of approximately 0.01 to 5% by mass based on the mass of the total solid content of the image recording layer.

**<Higher Fatty Acid Derivatives>**

To prevent the inhibition of polymerization by oxygen, a higher fatty acid derivative such as behenic acid or behenic amide may be added such as it is allowed to be locally present on the surface of the image recording layer of the invention in the drying step after application. The higher fatty acid derivative is preferably contained in the image recording layer in an amount of approximately 0.1 to 10% by mass based on the mass of the total solid content of the image recording layer.

**<Plasticizer>**

A plasticizer may be contained in the image recording layer of the invention in order to improve in-machine development properties.

Preferable examples of the plasticizer include phthalates such as dimethyl phthalate, diethyl phthalate, dibutyl phthalate, diisobutyl phthalate, dioctyl phthalate, octyl capryl phthalate, dicyclohexyl phthalate, tridecyl phthalate, butyl benzyl phthalate, diisodecyl phthalate and diallyl phthalate; glycol esters such as dimethyl glycol phthalate, ethyl phthalyl ethyl glycolate, methyl phthalyl ethyl glycolate, butyl phthalyl butyl glycolate and triethylene glycol dicaprylate; phosphates such as tricresyl phosphate and triphenyl phosphate; fatty dibasic acid esters such as diisobutyl adipate, dioctyl adipate, dimethyl sebacate, dibutyl sebacate, dioctyl azelate and dibutyl maleate; polyglycidyl methacrylate, triethyl citrate, glycerin triacetyl ester and butyl laurate.

The plasticizer is preferably contained in the image recording layer in an amount of approximately 30% by mass or less based on the mass of the total solid content of the image recording layer.

**<Inorganic Fine Particles>**

The image recording layer of the invention may contain inorganic fine particles in order to improve the strength of a cured film in an image region and the in-machine development properties of a non-image region.

Examples of the inorganic fine particles include silica, alumina, magnesium oxide, titanium oxide, magnesium carbonate, calcium alginate and a mixture thereof. Even if these do not have an ability to convert light/heat, they can be used in reinforcement of a coating film and reinforcement of interfacial adhesiveness by surface roughening.

The average particle diameter of the inorganic fine particle is preferably 5 nm to 10  $\mu\text{m}$ , and more preferably 0.5  $\mu\text{m}$  to 3  $\mu\text{m}$ . In the above range, the inorganic fine particles can be dispersed stably in the image recording layer to sufficiently maintain the strength of a film on the image recording layer to form a non-image region hardly tinted during printing and excellent in hydrophilicity.

The inorganic fine particles described above are easily available as commercial products such as colloidal silica dispersion.

The inorganic fine particles may be contained in the image recording layer in an amount of preferably 20% by mass or less, and more preferably 10% by mass or less, based on the mass of the total solid content of the image recording layer.

**<Low-Molecular Hydrophilic Compound>**

The image recording layer of the invention may contain a hydrophilic low-molecular compound in order to improve in-machine development properties. Examples of the hydrophilic low-molecular compound include water-soluble organic compounds, for example, glycols such as ethylene glycol, diethylene glycol, triethylene glycol, propylene glycol, dipropylene glycol and tripropylene glycol and ether or ester derivatives thereof, polyhydroxy compounds such as glycerin and pentaerythritol, organic amines such as triethanol amine and diethanol amine monoethanol amine and salts thereof, organic sulfonic acids such as toluene sulfonic acid and benzene sulfonic acid and salts thereof, organic phosphonic acids such as phenyl phosphonic acid and salts thereof, organic carboxylic acids such as tartaric acid, oxalic acid, citric acid, malic acid, lactic acid, gluconic acid and amino acid and salts thereof.

**<Formation of the Image Recording Layer>**

The image recording layer of the invention may be formed by dispersing or dissolving the necessary components described above in a solvent to prepare a coating solution and then applying the coating solution. Examples of the solvent to be used include, but are not limited to, ethylene dichloride, cyclohexanone, methyl ethyl ketone, methanol, ethanol, propanol, ethylene glycol monomethyl ether, 1-methoxy-2-propanol, 2-methoxyethyl acetate, 1-methoxy-2-propyl acetate, dimethoxyethane, methyl lactate, ethyl lactate, N,N-dimethylacetamide, N,N-dimethyl-formamide, tetramethyl urea, N-methylpyrrolidone, dimethyl sulfoxide, sulfolane,  $\gamma$ -butyrolactone, toluene and water. These solvents are used alone or as a mixture thereof. The solid content is preferably 1 to 50% by mass in the coating solution.

Alternatively, the image recording layer can be formed by preparing a plurality of coating solutions having the same or different components dispersed or dissolved in the same or different solvents and applying and drying the solutions repeatedly several times.

The preferable coating amount (solid content) of the image recording layer on a substrate, obtained after coating and drying, varies depending on applications, but is generally preferably 0.3 to 3.0  $\text{g}/\text{m}^2$ . In this range, good sensitivity and excellent film-making property of the image recording layer can be achieved.

For coating, various methods can be used as necessary. Examples of the coating method include bar coating, rotational coating, spray coating, curtain coating, dip coating, air knife coating, blade coating and roll coating.

**<Substrate>**

The substrate used in the planographic printing plate precursor of the invention is not particularly limited insofar as it is a dimensionally stable plate. Examples thereof include paper, paper with plastics (e.g., polyethylene, polypropylene, polystyrene, etc.) laminated thereon, a metal plate (e.g., aluminum, zinc, copper, etc.), a plastic film (e.g., diacetate cellulose, triacetate cellulose, propionate cellulose, butyrate cellulose, acetate butyrate cellulose, nitrate cellulose, polyethylene terephthalate, polyethylene, polystyrene, polypropylene, polycarbonate, polyvinyl acetal, etc.), and paper or a plastic film having the above-described metal laminated or vapor-deposited thereon. The substrate is pref-

erably a polyester film or an aluminum plate. Especially, the aluminum plate is particularly preferable because it is excellent in dimensional stability and relatively inexpensive.

The aluminum plate is preferably a pure aluminum plate or an alloy plate based on aluminum containing a trace of different elements, or a plastics laminate disposed on a thin aluminum or aluminum alloy film. The different elements contained in the aluminum alloy include silicon, iron, manganese, copper, magnesium, chrome, zinc, bismuth, nickel, titanium, etc. The content of the different elements in the alloy is preferably up to 10% by weight. A pure aluminum plate is preferable in the invention, but because production of absolutely pure aluminum is difficult even by refining techniques, aluminum may contain a trace of different elements. The composition of the aluminum plate is not limited, and any aluminum plates made of known and conventionally used material can be used as necessary.

The thickness of the substrate is preferably about 0.1 to 0.6 mm, more preferably 0.15 to 0.4 mm, and particularly preferably 0.2 to 0.3 mm.

Before use, the aluminum plate is subjected preferably to surface treatment such as roughening treatment or anodizing treatment. By surface treatment, hydrophilicity can be easily improved and the adhesion between the image recording layer and the substrate can be easily secured. Before the surface of the aluminum plate is roughened, degreasing treatment with e.g. a surfactant, an organic solvent or an aqueous alkali solution is conducted as necessary for removal of rolling oil on the surface thereof.

The treatment of roughening the surface of the aluminum plate is conducted in various methods such as a method of mechanical surface roughening, a method of surface roughening by electrochemical dissolution of the surface and a method of chemical surface roughening by chemically and selectively dissolving the surface.

The method of mechanical surface roughening can make use of known techniques such as ball grinding, brush grinding, blast grinding and buff grinding.

Examples of the electrochemical roughening method include a method of roughening the surface in a hydrochloric acid- or nitric acid-containing electrolyte by use of alternating current or direct current. A method of using a mixed acid as described in JP-A No. 54-63902 can also be mentioned.

The aluminum plate thus surface-roughened is subjected as necessary to alkali etching treatment with an aqueous solution of potassium hydroxide, sodium hydroxide, etc. and then to neutralization treatment, which may be followed if necessary by anodizing treatment to improve abrasion resistance.

As the electrolyte for use in the anodizing treatment of the aluminum plate, various electrolytes for forming a porous oxide film can be used. Generally, sulfuric acid, hydrochloric acid, oxalic acid, chromic acid or a mixed acid thereof is used. The concentration of the electrolyte is determined suitably depending on the type of the electrolyte.

The conditions for the anodizing treatment are varied depending on the electrolyte used and cannot be generalized, but it is usually preferable that the concentration of the electrolyte is 1 to 80% by weight, the liquid temperature is 5 to 70°C., the current density is 5 to 60 A/dm<sup>2</sup>, the voltage is 1 to 100 V, and the electrolysis time is 10 seconds to 5 minutes. The amount of the anodized film is preferably 1.0 to 5.0 g/m<sup>2</sup>, and more preferably 1.5 to 4.0 g/m<sup>2</sup>. In this range, good printing durability and good mar resistance of a non-image part in the planographic printing plate can be achieved.

After the anodizing treatment described above is conducted, the surface of the aluminum plate is subjected to hydrophilization treatment. Examples of the hydrophilization treatment include an alkali metal silicate method described in U.S. Pat. Nos. 2,714,066, 3,181,461, 3,280,734 and 3,902,734. In this method, the substrate is dipped or electrolyzed in an aqueous solution of sodium silicate. In addition, a method of treatment with potassium fluorozirconate as disclosed in JP-B 36-22063 or a method of treatment with polyvinyl phosphonic acid as disclosed in U.S. Pat. Nos. 3,276,868, 4,153,461, and 4,689,272 is mentioned.

The central line average roughness of the substrate is preferably 0.10 to 1.2 µm. In this range, excellent adhesiveness to the image recording layer, excellent printing durability and excellent stain resistance can be achieved.

The color density of the substrate, in terms of reflection density, is preferably 0.15 to 0.65. In this range, excellent image-forming property by prevention of halation during exposure of an image to light and excellent plate checking property after development can be obtained.

#### <Back Coat Layer>

The substrate is subjected to surface treatment or provided with an under-coating layer, and can then be provided if necessary with a back coat layer on the back of the substrate.

The back coat is preferably a coating layer including metal oxides obtained by hydrolysis and polycondensation of organic polymer compounds described in JP-A No. 5-45885 and organic or inorganic metal compounds described in JP-A No. 6-35174. Among these coating layers, coating layers made of metal oxides obtained from silicon alkoxy compounds such as Si(OCH<sub>3</sub>)<sub>4</sub>, Si(OC<sub>2</sub>H<sub>5</sub>)<sub>4</sub>, Si(OC<sub>3</sub>H<sub>7</sub>)<sub>4</sub> and Si(OC<sub>4</sub>H<sub>9</sub>)<sub>4</sub> are particularly preferable because these starting materials are easily available inexpensively.

#### <Under-Coating Layer>

In the planographic printing plate precursor of the invention used in the planographic printing method of the invention, an under-coating layer may be arranged if necessary between the image recording layer and the substrate. Because the under-coating layer functions as a thermally insulating layer, heat generated upon exposure to light from an infrared laser can be efficiently utilized by preventing the heat from diffusing into the substrate, thus achieving higher sensitivity. Further, in-machine development properties can be improved by facilitating release of the image recording layer from the substrate.

Examples of the material of the under-coating layer include a silane coupling agent having an addition-polymerizable ethylenically double bond reactive group described in JP-A No. 10-282679 and a phosphorus compound having an ethylenically double bond reactive group.

The coating amount (solid content) of the under-coating layer is preferably 0.1 to 100 mg/m<sup>2</sup>, and more preferably 3 to 30 mg/m<sup>2</sup>.

#### <Protective Layer>

In the planographic printing plate precursor of the invention used in the planographic printing method of the invention, a protective layer can be arranged on the image recording layer if necessary for preventing marring on the image recording layer, for shielding the image recording layer from oxygen and for preventing abrasion during exposure to light from a high-intensity laser.

In the invention, light exposure is conducted usually in the air, and by the protective layer, low-molecular compounds in

the air, such as oxygen, basic substances, etc. inhibiting an image formation reaction in the image recording layer initiated upon exposure to light, can be prevented from being introduced into the image recording layer, and thus prevented from inhibiting the image formation reaction upon exposure to light in the air. Accordingly, the protective layer has preferably such properties that the protective layer does not allow low-molecular compounds such as oxygen to permeate therethrough, but allows light used in light exposure to permeate sufficiently therethrough, is excellent in adhesion to the image recording layer, but can be removed easily in the development step on machine after exposure to light. The protective layer having such properties has been extensively examined and described in detail in U.S. Pat. No. 3,458,311 and JP-A No. 55-49729.

The materials used in the protective layer are preferably water-soluble polymer compounds relatively excellent in crystallinity. Specific examples include water-soluble polymers such as polyvinyl alcohol, polyvinyl pyrrolidone, acidic celluloses, gelatin, gum arabic and polyacrylic acid. Among these compounds, polyvinyl alcohol (PVA) can be used as a major component to provide the best result to basic characteristics such as oxygen impermeability and removability by developer. The polyvinyl alcohol may be partially replaced by ester, ether and acetal and may partially have other copolymerizable components insofar as it has unsubstituted vinyl alcohol units for giving necessary oxygen impermeability and water solubility. Particularly, a mixture containing polyvinyl alcohol replaced in the range of 15 to 50 wt % by polyvinyl pyrrolidone is preferable in view of shelf stability.

Examples of the polyvinyl alcohol include those hydrolyzed at a degree of 71 to 100%, having a polymerization degree in the range of 300 to 2400. Specific examples include PVA-105, PVA-110, PVA-117, PVA-117H, PVA-120, PVA-124, PVA-124H, PVA-CS, PVA-CST, PVA-HC, PVA-203, PVA-204, PVA-205, PVA-210, PVA-217, PVA-220, PVA-224, PVA-217EE, PVA-217E, PVA-220E, PVA-224E, PVA-405, PVA-420, PVA-613 and L-8, all of which are available from Kuraray Co., Ltd.

The components (PVA selected and additives used) in the protective layer, the coating amount, etc. are selected in consideration of fogging property, adhesiveness and anti-scratch property in addition to oxygen impermeability and removability by developer. In general, as the degree of hydrolysis of PVA is increased (or the content of unsubstituted vinyl alcohol units in the protective layer is increased) or as the thickness of the layer is increased, oxygen impermeability is increased to improve sensitivity. However, it is preferable for oxygen impermeability not to be extremely increased, in order to inhibit undesired polymerization reaction during production or storage or unnecessary fogging and dot gain upon exposure of an image to light. Accordingly, the oxygen permeability at 25° C. at 1 atmospheric pressure is preferably  $0.2 \leq A \leq 20$  (ml/m<sup>2</sup> day).

As other components in the protective layer, glycerine, dipropylene glycol, etc. can be added in an amount of a few wt % based on the (co)polymer, to confer flexibility, and anionic surfactants such as sodium alkylbenzenesulfonate and sodium alkylsulfonate, amphoteric surfactants such as alkylaminocarboxylates and alkylaminodcarboxylates and nonionic surfactants such as polyoxyethylene alkyl phenyl ether can be added in an amount of a few wt % based on the (co)polymer.

The thickness of the protective layer is suitably 0.1 to 5  $\mu\text{m}$ , particularly preferably 0.2 to 2  $\mu\text{m}$ .

In addition, adhesiveness to an image region and anti-scratch property are also very important for handling of the planographic printing plate precursor. That is, when the protective layer rendered hydrophilic by incorporating a water-soluble polymer is laminated on the image recording layer that is a lipophilic polymer layer, the protective layer is easily released due to insufficient adhesion so that the planographic printing plate precursor may undergo deficiency such as insufficient curing in the released portion because of the inhibition of polymerization by oxygen.

In response to this problem, various proposals for improving the adhesiveness between the image recording layer and the protective layer have been made. For example, JP-A No. 49-70702 and GB Patent Application Publication No.

15 1303578 describe that an acrylic emulsion, a water-insoluble vinyl pyrrolidone/vinyl acetate copolymer, etc. are mixed in an amount of 20 to 60% by weight in a hydrophilic polymer based on polyvinyl alcohol and then laminated on an image recording layer, thereby achieving satisfactory adhesiveness.

20 Any of these known techniques can be used in the invention. The method of applying the protective layer is described in detail in e.g. U.S. Pat. No. 3,458,311 and JP-A No. 55-49729.

Further, the protective layer can be endowed with other 25 functions. For example, a coloring agent (for example, a water-soluble dye) which is excellent in an ability to allow infrared rays used in light exposure to permeate therethrough and capable of efficiently absorbing lights of other wavelengths can be added to improve safelight suitability without deteriorating sensitivity.

#### [Planographic Printing Method]

Now, the planographic printing method using the planographic printing plate precursor of the invention is described 35 in detail. The planographic printing method of the invention comprises: providing a planographic printing plate precursor comprising a substrate and an image recording layer which is disposed on the substrate; imagewise exposing the planographic printing plate precursor with an infrared laser; and 40 supplying oil-based ink and an aqueous component to the exposed planographic printing plate precursor without any development treatment, so as to print an image. A region of the planographic printing plate precursor that has not been exposed with an infrared laser is removed during the printing.

45 Hereinafter, the method is described in the order of the steps.

#### [Light Exposure]

50 In the planographic printing method of the invention, the planographic printing plate precursor of the invention is first subjected to imagewise exposure to light with an infrared laser.

The infrared laser used in the invention is not particularly 55 limited, and is preferably a solid laser or a semiconductor laser emitting infrared rays of wavelengths of 760 to 1200 nm. The output power of the infrared laser is preferably 100 mW or more. A multi-beam laser device is preferably used to reduce the light exposure time.

60 The light exposure time per pixel is preferably within 20 micro seconds. The irradiation energy is preferably 10 to 300 mJ/m<sup>2</sup>.

#### [Printing]

65 In the planographic printing method of the invention, the planographic printing plate precursor of the invention is subjected to imagewise exposure to light with an infrared

75

laser and then used in printing by supplying oil ink and an aqueous component without any development treatment step.

Specifically, mention is made of a method which comprises exposing the planographic printing plate precursor to light with an infrared laser, and then fitting it into a printing machine to print an image without a development step and a method wherein the planographic printing plate precursor is fitted into a printing machine and exposed to light with an infrared laser in the printing machine to print an image without a development step.

When the planographic printing plate precursor is subjected to imagewise exposure to light with an infrared laser and then used in printing with an aqueous component and oil-based ink without a development treatment step such as a wet development treatment step, the image recording layer cured by exposure to light forms an oil-based ink receiving part having a lipophilic surface in the region of the image recording layer exposed to light. In the region not exposed to light, on the other hand, the green image recording layer is removed by dissolution or dispersion with the supplied aqueous component and/or oil-based ink, to permit a hydrophilic surface to be exposed on that region.

As a result, the aqueous component adheres to the exposed hydrophilic surface, while the oil-based ink adheres to the image region in the light-exposed region to initiate printing. The component to be first added may be the aqueous component or oil-based ink, but preferably the oil-based ink is first added in order to prevent the aqueous component from being polluted with the image recording layer in the region not exposed to light. As the aqueous component and oil-based ink, conventional planographic dampening water and printing ink are used.

The planographic printing plate precursor is developed on an offset printing machine and used in printing to produce a large number of prints.

The image recording layer in the planographic printing plate precursor of the invention is excellent in curing properties of the light-exposed region and printing durability, and can be rapidly cured upon exposure to light with an infrared laser to form a strong ink receiving region even in an image region of small area such as halftone dot, while owing to the high solubility and dispersibility, with dampening water and/or ink, of the image recording layer, the region not exposed to light is removed easily in a short time upon contacting with dampening water and/or ink, and thus the planographic printing plate precursor can exhibit a significant effect upon application to the planographic printing method of the invention where no special development treatment is conducted.

## EXAMPLES

Hereinafter, the present invention is described in detail by reference to the Examples. However, the following examples should not be construed to limit the scope of the invention.

### 1. Preparation of a Planographic Printing Plate Precursor

#### (1) Preparation of a Substrate

##### <Aluminum Plate>

A melt of a JIS A1050 aluminum alloy containing 99.5 wt % or more aluminum, 0.30 wt % Fe, 0.10 wt % Si, 0.02 wt % Ti, and 0.013 wt % Cu was subjected to cleaning treatment and then cast. In this cleaning treatment, the melt was degassed to remove unnecessary gas such as hydrogen,

76

and filtered through a ceramic tube filter. Casting was conducted using a DC casting method. After 10-mm surface layer was removed from the coagulated ingot plate of 500 mm in thickness, the plate was subjected to homogenization treatment at 550° C. for 10 hours so that intermetallic compounds were not agglomerated. Then, the plate was hot-rolled at 400° C., then annealed at 500° C. for 60 seconds in a continuous annealing furnace and cold-rolled to form an aluminum rolled plate of 0.30 mm in thickness. By regulating the roughness of pressure rollers, the central line average surface roughness Ra after cold rolling was regulated to be 0.2 µm. Thereafter, the plate was placed in a tension leveler to improve flatness. The resulting aluminum plate was subjected to the following surface treatment.

First, the surface of the aluminum plate was degreased at 50° C. for 30 seconds in 10 wt % aqueous sodium aluminate to remove the rolling oil therefrom and then neutralized with 30 wt % aqueous nitric acid at 50° C. for 30 seconds, to remove smuts therefrom.

Then, the surface of the substrate was roughened, thereby facilitating the adhesion of the substrate to an image recording layer while conferring water holding property on a non-image region. Specifically, the aluminum plate was subjected to electrochemical surface roughening treatment through electrolysis of the aluminum plate by passing the aluminum plate web in an aqueous solution containing 1 wt % nitric acid and 0.5 wt % aluminum nitrate (solution temperature, 45° C.) supplied into an indirect feeder cell at an electricity of 240 C/dm<sup>2</sup> at the side of an anode at a current density of 20 A/dm<sup>2</sup> in an alternating waveform in the duty ratio of 1:1.

Further, the aluminum plate was etched at 35° C. for 30 seconds in 10 wt % aqueous sodium hydroxide and then neutralized with 30 wt % aqueous sulfuric acid at 50° C. for 30 seconds to remove smuts therefrom.

Thereafter, the aluminum plate was subjected to anodizing treatment to improve abrasion resistance, chemical resistance and water holding property. Specifically, the plate was subjected to electrolysis by passing the aluminum plate web in 20 wt % aqueous sulfuric acid (solution temperature, 35° C.) supplied into an indirect feeder cell at a direct current of 14 A/dm<sup>2</sup>, to form 2.5 g/m<sup>2</sup> anodized film thereon.

Thereafter, the surface of the substrate was subjected to silicate treatment with 1.5 wt % aqueous sodium silicate solution No. 3 at 70° C. for 15 seconds in order to secure hydrophilicity on a non-image region. The amount of Si adhering thereto was 10 mg/m<sup>2</sup>. The substrate was washed with water. The central line surface roughness Ra of the resulting substrate was 0.25 µm.

#### (2) Formation of an Image Recording Layer

##### Example 1

The above substrate was coated by a bar with an image recording layer coating solution having the following composition and then dried in an oven at 70° C. for 60 seconds, to form an image recording layer having a coating amount of 0.8 g/m<sup>2</sup> after drying, whereby a planographic printing plate precursor was obtained.

##### Image recording layer coating solution (1)

|                                            |       |
|--------------------------------------------|-------|
| Water                                      | 100 g |
| Microcapsules (1) below (as solid content) | 5 g   |

-continued

| Image recording layer coating solution (1) |       |
|--------------------------------------------|-------|
| Polymerization initiator (G-1) below       | 0.5 g |
| Fluorine-containing surfactant (1) below   | 0.2 g |



## (Synthesis of Microcapsules (1))

10 g trimethylol propane/xylene diisocyanate adduct [Takenate D-110N manufactured by Mitsui Takeda Chemical], 3.15 g pentaerythritol triacrylate (SR444 manufactured by Nippon Kayaku Co., Ltd.), 0.35 g infrared absorber (1) below, 1 g 3-(N,N-diethylamino)-6-methyl-7-anilinofluoran (ODB manufactured by Yamamoto Kasei) and 0.1 g Pionine A41C (manufactured by Takemoto Oil & Fat Co., Ltd.) were dissolved as oil-phase components in 17 g ethyl acetate. As the aqueous-phase component, 40 g of 4 wt % aqueous PVA-205 was prepared. The oil-phase components were mixed with the aqueous-phase component and then emulsified at 12000 rpm for 10 minutes with a homogenizer. Thereafter, the resulting emulsion was added to 25 g distilled water and stirred at room temperature for 30 minutes and then stirred at 40° C. for 3 hours. Thus obtained microcapsule liquid (1) was diluted with distilled water so that the solid content became 20 wt %. The average particle diameter of the microcapsules thus obtained was 0.3  $\mu\text{m}$ .



## Example 2 and Comparative Example 1

The planographic printing plate precursor in Example 2 was obtained in the same manner as in Example 1 except in that the polymerizable compound and polymerization initiator used were changed into the compounds shown in Table 1 below. The planographic printing plate precursor in Comparative Example 1 was obtained in the same manner as in Example 1 except in that the polymerizable compound to be used was changed to M-1 (polyethylene glycol diacrylate). The structure of the polymerization initiator (G-2) used in Example 2 is shown below.

15

TABLE 1

|             | Polymerizable compound | Polymerization initiator | Infrared absorber | Binder | Printing durability |
|-------------|------------------------|--------------------------|-------------------|--------|---------------------|
| Example 1   | II-(b)-(ii)-23         | G-1                      | (1)               | —      | 120                 |
| Example 2   | III-(b)-19             | G-2                      | (1)               | —      | 135                 |
| Comparative | M-1                    | G-1                      | (1)               | —      | 100                 |
| Example 1   |                        |                          |                   |        |                     |

30



45

## Examples 3 to 10 and Comparative Example 2

The same substrate as in Example 1 was coated by a bar with an image recording layer coating solution having the following composition and then dried in an oven at 100° C. for 60 seconds, to form an image recording layer having a coating amount of 1.0 g/m<sup>2</sup> after drying, whereby a planographic printing plate precursor was obtained.

55

## Image recording layer coating solution (2)

|                                                        |        |
|--------------------------------------------------------|--------|
| Infrared absorber (compound shown in the table)        | 0.05 g |
| Polymerization initiator (compound shown in the table) | 0.2 g  |
| Binder polymer (compound shown in the table)           | 0.5 g  |
| (Average molecular weight 80,000)                      |        |
| Polymerizable compound (compound shown in the table)   | 1.0 g  |
| Victoria Pure Blue naphthalene sulfonate               | 0.02 g |
| Fluorine-based surfactant (1) above                    | 0.1 g  |
| Methyl ethyl ketone                                    | 18.0 g |

60

65

TABLE 2

|                       | Polymerizable compound | Polymerization initiator | Infrared absorber | Binder | Printing durability |
|-----------------------|------------------------|--------------------------|-------------------|--------|---------------------|
| Example 3             | II-(b)-(i)-14          | G-1                      | IR-1              | BP-1   | 125                 |
| Example 4             | II-(b)-(iii)-10        | G-1                      | IR-2              | BP-1   | 120                 |
| Example 5             | III-(b)-19             | G-1                      | IR-1              | BP-2   | 130                 |
| Example 6             | IV- b -14              | G-1                      | IR-1              | BP-1   | 130                 |
| Example 7             | II-(b)-(i)-16/M-1      | G-1                      | IR-1              | BP-1   | 125                 |
| Example 8             | II-(b)-(iii)-12        | G-2                      | IR-1              | BP-1   | 120                 |
| Example 9             | II-(b)-18              | G-2                      | IR-2              | BP-1   | 135                 |
| Example 10            | IV-(b)-6               | G-2                      | IR-1              | BP-1   | 130                 |
| Comparative Example 2 | M-2                    | G-1                      | IR-1              | BP-2   | 100                 |

Infrared absorber (IR-1)



Infrared absorber (IR-2)



BP-1



BP-2

In Example 2, two kinds of polymerizable compounds shown in the table were added in a ratio of 1:1 by weight. The polymerizable compound used in Comparative Example 2 was M-2 (tetramethylol methane triacrylate).

The image recording layer of each planographic printing plate precursor obtained above was coated with 2 wt % aqueous polyvinyl alcohol (degree of saponification, 98 mol %; degree of polymerization, 550) so that the coating amount after drying was 0.7 g/m<sup>2</sup>, followed by drying at 100° C. for 50 seconds to form a planographic printing plate precursor having a protective layer formed thereon, and then the following evaluation was performed.

## 2. Light Exposure and Printing

The resulting planographic printing plate precursor was exposed to light under the conditions of a power of 9 W, an external drum revolution of 210 rpm and a resolution of

50 2400 dpi by Trendsetter 3244VX equipped with a water-cooling 40-W infrared semiconductor laser. 50% halftone dots were contained in the light-exposed image. The resulting precursor exposed to light was fitted, without development treatment, into a cylinder in a printing machine SOR-M manufactured by Heidelberg. It was supplemented with dampening water (EU-3 (etching solution manufactured by Fuji Photo Film Co., Ltd.)/water/isopropyl alcohol=1/89/10 (ratio by volume)) and TRANS-G (N) black ink (manufactured by Dainippon Ink and Chemicals, Inc.) and used in producing 100 prints at a speed of 6000 prints per hour.

60 After development, in the printing machine, of the region of the image recording layer not exposed to light was finished, the number of printing papers required until the ink could not be transferred to the printing paper was evaluated

## 81

as in-machine development properties. As a result, any planographic printing plate precursors in Examples 1 to 10 and Comparative Examples 1 and 2 could be used to provide 100 or less prints without smutting in the non-image region.

## 3. Evaluation

In the case of the negative-type planographic printing plate precursor, the degree of curing of the image recording layer (photosensitive layer) is low when the amount of exposure light is low, while the degree of curing is high when the amount of exposure light is high. When the degree of curing of the image recording layer is too low, the planographic printing plate is poor in printing durability and inferior in reproducibility of small dots and thin lines. On the other hand, when the degree of curing of the image recording layer is high, the planographic printing plate is superior in printing durability and excellent in reproducibility of small dots and thin lines.

As shown below, the negative-type planographic printing plate precursor obtained above was used in forming an image by exposure to the same amount of light as described above, to evaluate printing durability in 50% halftone-dot region.

The results of halftone dot printing durability are shown in Tables 1 and 2. As can be seen from Tables 1 and 2, the planographic printing plate obtained by the planographic printing method of the invention using the planographic printing plate precursor of the invention is superior in halftone dot printing durability as compared to the planographic printing plate precursor using a polymerizable compound which is outside of the scope of the invention. From the result of printing evaluation, it was confirmed that any planographic printing plate precursors of the invention are excellent in in-machine development properties.

What is claimed is:

1. A planographic printing method comprising: providing a planographic printing plate precursor comprising a substrate and an image recording layer which is disposed on the substrate and comprises (A) an infrared absorber, (B) a polymerization initiator and (C) a polymerizable compound, the image recording layer being capable of recording with irradiation of infrared rays; imagewise exposing the planographic printing plate precursor with an infrared laser; and supplying oil-based ink and an aqueous component to the exposed planographic printing plate precursor without any development treatment, so as to print an image, wherein a region of the planographic printing plate precursor that has not been exposed with an infrared laser is removed during the printing, and the polymerizable compound of (C) is represented by the following formula (1):



Formula (1)

## 82

wherein Ar¹ represents an arylene group or a divalent heterocyclic group; R¹ represents a hydrogen atom or an alkyl group having 1 to 6 carbon atoms; Z represents an n-valent organic linking group; and n denotes an integer of 1 to 20.

2. The planographic printing method of claim 1, wherein the polymerization initiator of (B) is an onium salt.

3. The planographic printing method of claim 1, wherein the image recording layer further comprises (D) a binder polymer.

4. The planographic printing method of claim 1, wherein the image recording layer further comprises (F) microcapsules.

5. The planographic printing method of claim 4, wherein the microcapsules incorporate at least one of the components contained in the image recording layer.

6. The planographic printing method of claim 1, wherein Ar¹ represents a phenylene group.

7. The planographic printing method of claim 1, wherein R¹ represents a methyl group or an ethyl group.

8. The planographic printing method of claim 1, wherein Z represents an n-valent organic linking group containing at least one of the following groups:



9. The planographic printing method of claim 1, wherein in Ar¹, CH₂=CR¹— is located at a para-position with respect to Z—.

10. A planographic printing plate precursor comprising a substrate and an image recording layer which is disposed on the substrate and comprises (A) an infrared absorber, (B) a polymerization initiator, and (C) a polymerizable compound, the image recording layer being removable with printing ink and/or dampening water,

wherein the polymerizable compound of (C) is represented by the following formula (1):



Formula (1)

wherein Ar¹ represents an arylene group or a divalent heterocyclic group; R¹ represents a hydrogen atom or an alkyl group having 1 to 6 carbon atoms; Z represents an n-valent organic linking group; and n denotes an integer of 2 to 20.

11. The planographic printing plate precursor of claim 10, wherein the polymerization initiator of (B) is an onium salt.

12. The planographic printing plate precursor of claim 10, wherein the image recording layer further comprises (D) a binder polymer.

**83**

13. The planographic printing plate precursor of claim 10, wherein the image recording layer further comprises (F) microcapsules.

14. The planographic printing plate precursor of claim 13, 5 wherein the microcapsules incorporate at least one of the components contained in the image recording layer.

15. The planographic printing plate precursor of claim 10, 10 wherein Ar<sup>1</sup> represents a phenylene group.

16. The planographic printing plate precursor of claim 10, wherein R<sup>1</sup> represents a methyl group or an ethyl group.

**84**

17. The planographic printing plate precursor of claim 10, wherein Z represents an n-valent organic linking group containing at least one of the following groups:



18. The planographic printing plate precursor of claim 10, wherein in Ar<sup>1</sup>,  $\text{CH}_2=\text{CR}^1-$  is located at a para-position with respect to Z.

\* \* \* \* \*